# EUROPEAN PATENT SPECIFICATION

(11) **EP 4 143 279 B1**
(45) Date of publication and mention of the grant of the patent: **26.06.2024**
(21) Application number: 21720541.8
(22) Date of filing: 28.04.2021
(51) Int. Cl.: C10M 145/14

(54) **PROCESS FOR THE PREPARATION OF DISPERSANT POLYALKYL (METH)ACRYLATE POLYMERS**
VERFAHREN ZUR HERSTELLUNG VON DISPERGIERENDEN POLYALKYL(METH)ACRYLATPOLYMEREN
PROCÉDÉ POUR LA PRÉPARATION DE POLYMÈRES POLY(MÉTH)ACRYLATES D'ALKYLE DISPERSANTS

(30) Priority: 30.04.2020 EP 20172357
(43) Date of publication of application: 08.03.2023
(73) Proprietor: Evonik Operations GmbH, 45128 Essen (DE)
(72) Inventor: SCHÖLLER, Katrin, 65812 Bad Soden (DE); ZIEGLER, Fabian, 64289 Darmstadt (DE); TSCHEPAT, Wolfgang, 64291 Darmstadt (DE); LIPPERT, Sarah, 64285 Darmstadt (DE); DOERFEL, Mara, 64823 Groß-Umstadt (DE)
(74) Representative: Evonik Patent Association
(86) International application number: PCT/EP2021/061045
(87) International publication number: WO 2021/219679

(56) References cited:
- EP-A1- 3 450 527
- WO-A1-2018/041755

## Description

The present invention is directed to a novel process for the preparation of polyalkyl (meth)acrylate polymers with improved compositional distribution leading to better producibility, solubility and improved performance of the products in lubricant compositions, especially in engine oil formulations.

Lubricants are playing an important role in reducing a vehicle's fuel consumption and there is a continuing need for improvements in fuel economy performance.

Formulations of motor oils are generally defined by the SAE J300 standard (SAE = Society of Automotive Engineers). This standard classifies motor oils into the SAE viscosity grades xW-y where x = 0, 5, 10, 15, 20, 35 and y = 8, 12, 16, 20, 30, 40, 50, 60. This is done e.g. via the kinematic viscosity KV (ASTM D445) and the high-temperature high-shear viscosity HTHS (ASTM D4683, D4741 and D5471), which parameters are important for engine protection.

Lubricant properties are typically improved by the addition of additives to lubricating oils. Viscosity index (VI) improvers are generally added to a lubricant to improve its thickening efficiency and to protect the engine.

In the past decade, a lot of efforts were taken to improve lubricants towards better fuel efficiency.

Polyalkyl (meth)acrylate-based polymers, and especially polyalkyl (meth)acrylates comprising macromonomers, are commonly used as additives, especially as viscosity index improvers. They show good viscometric properties like low KV₄₀, HTHS₈₀ and HTHS₁₀₀ values in engine oil formulations leading to good fuel economy.

Polyalkyl (meth)acrylate polymers usually comprise short-chain alkyl (meth)acrylates and long-chain alkyl (meth)acrylates. Short-chain alkyl (meth)acrylates are more polar and contribute to the viscometric properties of the resulting polymer, whereas long-chain alkyl (meth)acrylates are less polar and provide the oil solubility of the resulting polymer.

The composition of a polyalkyl (meth)acrylate has to be well balanced between polar and apolar monomers as a raise in polarity usually comes along with poor solubility and an undesired change in the viscometric performance of the polymer.

Adding a high number of polar monomers like methyl (meth)acrylate (MMA), butyl (meth)acrylate (BMA), styrene or functional monomers like dimethylaminoethyl methacrylate (DMAEMA) to polyalkyl (meth)acrylates and specifically to polyalkyl (meth)acrylates comprising macromonomers leads to the technical problem that the polarity of the polymer is increased too much leading to a changed viscosity and in general a poorer solubility of the polymer in oil.

One typical approach to counteract this polarity increase is to balance the polymer polarity by increasing the amount of less polar comonomers like for example long-chain alkyl (meth)acrylates or macromonomers. Although the solubility of the polymer in oil can be improved this way, the drawback of this approach is that the viscometric performance measured as KV₄₀, HTHS₈₀, or HTHS₁₀₀ values in oil is compromised. This means that increasing for example the amount of long-chain alkyl (meth)acrylates leads to an increased KV₄₀, HTHS₈₀ and HTHS₁₀₀ and therefore reduced fuel efficiency effect.

The comb polymer technology in general and their use as viscosity index improvers is already known in the art (US 2008/0194443 and US 2010/0190671).

The viscometric performance of a polyalkyl (meth)acylate based comb polymer can e.g. be improved by introducing novel monomers. It is already known in the art that a certain amount of macromonomers has a positive impact on fuel efficiency (US 2010/0190671), that the presence of alkyl acrylates improves the NOACK volatility (WO 2018/041755) and a certain amount of imide functionality has a positive impact on friction reduction (WO 2019/012031).

Another challenge that usually comes along with a reduced solubility and the polymer becoming too polar is that the polymer's producibility and especially up-scalability in the plant might be hindered. Possible results are, for example, an immense increase in haziness in the product, increased in-process viscosities, increased heat-generation and/or the building of non-soluble deposits. Each of these drawbacks can hinder the production of such a product or do at least lead to an economically not favorable production process, where a continuous run is not possible leading to shorter production cycles with extensive and costly cleaning steps of the production kettle after each production batch.

It was therefore an object of the present invention to provide polyalkyl (meth)acrylates wherein the polarity of the polymer is increased as much as possible to improve or keep good KV₄₀, HTHS₈₀ and HTHS₁₀₀ performance and, at the same time, provide good solubility, up-scalability and economic producibility.

It was surprisingly found that a novel method for producing polyalkyl (meth)acrylates, wherein the amounts of the different monomers are split into a heel and one or more feeds with different compositions and concentrations, results in polymer compositions that are better balanced, i.e. leads to the formation of a higher amount of polymers having a composition closer to the average polymer composition throughout the whole polymerization process.

This approach leads to products with improved solubility, reduced HAZE (marker for the solubility of the polymer in a given base oil) and reduced deposits formation in the reactor, improved up-scalability and very good viscometric properties at the same time.

The changed process conditions additionally allow the synthesis of new polymer compositions with improved viscometric properties towards fuel efficiency that were not producible before and showed an unfavorable solubility in oil.

### State of the art

The processes known in the art for the preparation of polyalkyl (meth)acrylates are all based on the reaction of a mixture comprising the monomers in the ratios as desired for the resulting polymer(s). These mixtures are either reacted in a one-pot reaction after addition of initiator or they are split into a heel and a feed which do both have exactly the same composition.

US 2008/0194443 and US 2010/0190671 disclose a synthesis of comb polymers wherein a mixture of all monomers is added to an apparatus and diluted with base oil. Subsequently, the reaction mixture is heated to a desired temperature and reacted while several shots of initiator are added after certain time intervals. A split of the monomers into different feeds with different compositions and concentrations of monomers is not mentioned.

US 2011/0306533 and US 2011/0319305 disclose a method for the preparation of comb polymers wherein an initial reaction mixture is prepared comprising all of the monomers and solvent oil. This initial reaction mixture is then split into a heel (about one fifth of the initial reaction mixture) and a feed (about four fifth of the initial reaction mixture). The compositions of the monomers in both, heel and feed are the same as well as are the concentrations of the monomers. After reaching the reaction temperature, several shots of initiator are added after certain time intervals. A split of the monomers into different feeds with different compositions and concentrations of monomers is not mentioned.

WO 2014/170169 discloses a method for the preparation of comb polymers wherein an initial reaction mixture is prepared comprising all the monomers and solvent oil. This initial reaction mixture is then split into a heel (about one third of the initial reaction mixture) and a feed (about two thirds of the initial reaction mixture). The compositions of the monomers in both, heel and feed are the same as well as are the concentrations of the monomers. After reaching the reaction temperature, several shots of initiator are added after certain time intervals. A split of the monomers into different feeds with different compositions and concentrations is not mentioned.

WO 2019/012031 is directed to comb polymers and describes a base polymer synthesis wherein an apparatus is initially charged with a mixture of 300 g of monomers and 200 g of solvent oil. This mixture is heated, and initiator added. Subsequently, another mixture of 300 g of monomers and 200 g of solvent oil, having the same composition and concentration as the initial mixture, is added as a feed as well as further initiator shot. A split of the monomers into different feeds with different compositions and concentrations of monomers is not mentioned.

WO 2018/114673 discloses a method for the preparation of comb polymers wherein an initial reaction mixture of different monomers and solvent oil is prepared. 50% of said mixture are charged into a beaker and the other 50% of the initial mixture fed during a time interval. Monomer composition and concentration are the same. Several shots of initiator are added after certain time intervals. A split of the monomers into different feeds having different compositions and concentrations is not mentioned.

WO 2018/041755 discloses a method for the preparation of comb polymers wherein a heel is charged with an initial mixture of monomers and solvent oil and a feed of monomers in solvent is added. The composition of the monomers in heel and feed are the same, but the concentrations of heel and feed are different.

### Detailed description of the invention

According to the literature, the monomers generally used to prepare polyalkyl (meth)acrylate polymers do not differ significantly in their Q,e-parameters (Q = reactivity, e = polarity). That means that the person skilled in the art would not expect any difficulties for the copolymerization of different monomers having similar Q,e-parameters. Following the description of the existing polymerization models, only for sterically hindered monomers the kinetics cannot be easily forecasted or calculated.

Copolymerization parameters need to be defined for each comonomer couple individually and temperature, medium and initiator need to be considered as well because the copolymerization parameters are parameters for the relative reactivity only. In systems where the copolymerization parameters of such a monomer A-monomer B couple differ significantly, the first synthesized polymer molecules show a different composition than the later polymerized ones. Partial demixing is therefore a known phenomenon occurring for such polymer mixtures. Copolymers with constant composition over time can then be obtained by adding the faster polymerizing monomer according to its conversion or working at azeotrope conditions. In technical copolymerizations and products where many comonomers are applied this becomes challenging.

Q,e-parameters allow for an estimation of unknown copolymerization parameters. Similar e-values lead to azeotrope polymers while different e-values lead to alternating copolymers. For some comonomers it is difficult to forecast its copolymerization, especially for sterically hindered monomers or for such that cannot copolymerize.

In systems comprising macromonomers, the kinetics of all monomer couples can become really complicated. It was therefore a surprising finding for the skilled person that simply separating the polar monomers from the apolar (= oil-soluble) monomers was sufficient to get polymers with more uniform distribution and with much better solubility and viscometric performance than those prepared without splitting. This approach is more efficient and easier to implement than checking the reactivity (in oil) plus taking radical concentrations throughout the reaction into account as commonly suggested in the literature.

The described new process can be applied to all free radical polymerizations run in a feed process wherein at least one comonomer exhibits a copolymerization kinetics that varies significantly from the kinetics of the other comonomers.

In principle, all kinds of polyalkyl (meth)acrylates comprising monomers that show differences in polarity, reactivity and oil solubility can be prepared by the process according to the present invention.

A first object of the present invention is therefore directed to a method for the preparation of polyalkyl (meth)acrylate polymers consisting of:
(a) 10 to 20% by weight of esters of (meth)acrylic acid and a hydroxylated hydrogenated polybutadiene;
(b1) 45% to 60% by weight of C₁₋₄ alkyl (meth)acrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N-containing monomers selected from the group consisting of N,N-dimethylaminoethyl methacrylate (DMAEMA), N-(3-(dimethylamino)propyl)methacrylamide (DMAPMAm) and N-vinylpyrrolidinone (NVP), preferably DMAEMA, the method comprising the steps of:
   (i) preparing a monomer mixture **1** comprising 130 to 145% of the targeted content of monomers (a) and 90% to 96% of the targeted content of monomers (b), the concentration of the monomers in mixture **1** being 50 to 60%;
   (ii) adding a monomer mixture **2** comprising 50 to 60% of the targeted content of monomers (a) and 105% to 110% of the targeted content of monomers (b), the concentration of the monomers in mixture **2** being 50 to 60%;
characterized in that monomer mixture **1** comprises 50 to 60% of the total amount of monomers used in the process and monomer mixture **2** comprises 40 to 50% of the total amount of monomers used in the process.

A further first object of the present invention is directed to the method for the preparation of polyalkyl (meth)acrylate polymers as described further above, wherein the monomer mixture **2** can be further split into monomer mixture **2a** and monomer mixture **2b,** wherein
mixture **2a** comprises 100% of the targeted content of monomers (a) and 100% of the targeted content of monomers (b), the concentration of the monomers in mixture **2a** being 50 to 60% and
monomer mixture **2b** comprises 0% of the targeted content of monomers (a) and 115-125% of the targeted content of monomers (b), the concentration of the monomers in mixture **2b** being 50 to 60%,
characterized in that monomer mixture **2a** comprises 20 to 30% of the total amount of monomers used in the process, and monomer mixture **2b** comprises 20 to 25% of the total amount of monomers used in the process.

A further first object is directed to the method as described further above, wherein the polyalkyl (meth)acrylate polymer consists of:
(a) 10 to 20% by weight of esters of (meth)acrylic acid and a hydroxylated hydrogenated polybutadiene;
(b1) 45% to 60% by weight of C₁₋₄ alkyl methacrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N,N-dimethylaminoethyl methacrylate (DMAEMA).

The content of each component (a), (b1), (b2), (b3) and (b4) is based on the total composition of the polyalkyl (meth)acrylate polymer.

In a particular embodiment, the proportions of components (a), (b1), (b2), (b3) and (b4) add up to 100% by weight.

The weight-average molecular weight of the polyalkyl(meth)acrylate polymers according to the present invention is preferably in the range of 100,000 to 1,000,000 g/mol, more preferably in the range of 400,000 to 700,000 g/mol. The number-average molecular weight of the polyalkyl(meth)acrylate polymers according to the present invention is preferably in the range of 60,000 to 300,000 g/mol, more preferably in the range of 100,000 to 200,000 g/mol.

Preferably, the polyalkyl(meth)acrylate polymers according to the present invention have a polydispersity index (PDI) M_{w}/Mₙ in the range of 2 to 10, more preferably in the range of 2 to 6. M_{w} and Mₙ are determined by size exclusion chromatography (SEC) using commercially available polymethylmethacrylate standards. The determination is affected by gel permeation chromatography with THF as eluent.

A polyalkyl(meth)acrylate polymer in the context of this invention comprises a first polymer, which is also referred to as backbone or main chain, and a multitude of further polymers which are referred to as side chains and are bonded covalently to the backbone. In the present case, the backbone of the polyalkyl(meth)acrylate polymer is formed by the interlinked unsaturated groups of the mentioned (meth)acrylates. The ester groups of the (meth)acrylic esters, the phenyl radicals of the styrene monomers and the substituents of the further free-radically polymerizable comonomers form the side chains of the comb polymer.

The term "(meth)acrylate" refers to both, esters of acrylic acid and esters of methacrylic acid. Methacrylates are preferred over acrylates.

Polyolefin-based macromonomers comprise at least one group which is derived from polyolefins. Polyolefins are known in the technical field and can be obtained by polymerizing alkenes and/or alkadienes which consist of the elements carbon and hydrogen, for example C2-C10-alkenes such as ethylene, propylene, n-butene, isobutene, norbornene, and/or C4-C10-alkadienes such as butadiene, isoprene, norbornadiene. The repeating units derived from polyolefin-based macromonomers comprise preferably at least 70% by weight and more preferably at least 80% by weight and most preferably at least 90% by weight of groups which are derived from alkenes and/or alkadienes, based on the weight of the repeating units derived from polyolefin-based macromonomers. The polyolefinic groups may in particular also be present in hydrogenated form. In addition to the groups which are derived from alkenes and/or alkadienes, the repeating units derived from polyolefin-based macromonomers may comprise further groups. These include small proportions of copolymerizable monomers. These monomers are known per se and include, among other monomers, alkyl (meth)acrylates, styrene monomers, fumarates, maleates, vinyl esters and/or vinyl ethers. The proportion of these groups based on copolymerizable monomers is preferably at most 30% by weight, more preferably at most 15% by weight, based on the weight of the repeat units derived from polyolefin-based macromonomers. In addition, the repeating units derived from polyolefin-based macromonomers may comprise starting groups and/or end groups which serve for functionalization or are caused by the preparation of the repeat units derived from polyolefin-based macromonomers. The proportion of these starting groups and/or end groups is preferably at most 30% by weight, more preferably at most 15% by weight, based on the weight of the repeat units derived from polyolefin-based macromonomers.

Preferred polyolefin-based macromonomers are esters of (meth)acrylic acid and a hydroxylated hydrogenated polybutadiene.

The hydroxylated hydrogenated polybutadiene for use in accordance with the invention has a number-average molar mass Mₙ of 4,000 to 6,000 g/mol, preferably 4,500 to 5,000 g/mol. Because of their high molar mass, the hydroxylated hydrogenated polybutadienes can also be referred to as macroalcohols in the context of this invention.

The number-average molar mass Mₙ is determined by size exclusion chromatography using commercially available polybutadiene standards. The determination is affected to DIN 55672-1 by gel permeation chromatography with THF as eluent.

Preferably, the hydroxylated hydrogenated polybutadiene has a hydrogenation level of at least 99%. An alternative measure of the hydrogenation level which can be determined on the copolymer of the invention is the iodine number. The iodine number refers to the number of grams of iodine which can be added onto 100 g of copolymer. Preferably, the copolymer of the invention has an iodine number of not more than 5 g of iodine per 100 g of copolymer. The iodine number is determined by the Wijs method according to DIN 53241-1:1995-05.

Preferred hydroxylated hydrogenated polybutadienes can be obtained according to GB 2270317.

Preference is given to monohydroxylated hydrogenated polybutadienes. More preferably, the hydroxylated hydrogenated polybutadiene is a hydroxyethyl- or hydroxypropyl-terminated hydrogenated polybutadiene. Particular preference is given to hydroxypropyl-terminated polybutadienes.

These monohydroxylated hydrogenated polybutadienes can be prepared by first converting butadiene monomers by anionic polymerization to polybutadiene. Subsequently, by reaction of the polybutadiene monomers with ethylene oxide or propylene oxide, a hydroxy-functionalized polybutadiene can be prepared. This hydroxylated polybutadiene can be hydrogenated in the presence of a suitable transition metal catalyst.

The esters of (meth)acrylic acid for use in accordance with the invention and a hydroxylated hydrogenated polybutadiene described are also referred to as macromonomers in the context of this invention because of their high molar mass.

The macromonomers for use in accordance with the invention can be prepared by transesterification of alkyl (meth)acrylates. Reaction of the alkyl (meth)acrylate with the hydroxylated hydrogenated polybutadiene forms the ester of the invention. Preference is given to using methyl (meth)acrylate or ethyl (meth)acrylate as reactant.

This transesterification is widely known. For example, it is possible for this purpose to use a heterogeneous catalyst system, such as lithium hydroxide/calcium oxide mixture (LiOH/CaO), pure lithium hydroxide (LiOH), lithium methoxide (LiOMe) or sodium methoxide (NaOMe) or a homogeneous catalyst system such as isopropyl titanate (Ti(OiPr)₄) or dioctyltin oxide (Sn(OCt)₂O). The reaction is an equilibrium reaction. Therefore, the low molecular weight alcohol released is typically removed, for example by distillation.

In addition, the macromonomers can be obtained by a direct esterification proceeding, for example, from (meth)acrylic acid or (meth)acrylic anhydride, preferably under acidic catalysis by p-toluenesulfonic acid or methanesulfonic acid, or from free methacrylic acid by the DCC method (dicyclohexylcarbodiimide).

Furthermore, the present hydroxylated hydrogenated polybutadiene can be converted to an ester by reaction with an acid chloride such as (meth)acryloyl chloride.

Preferably, in the above-detailed preparations of the esters of the invention, polymerization inhibitors are used, for example the 4-hydroxy-2,2,6,6-tetramethylpiperidinooxyl radical and/or hydroquinone monomethyl ether.

The C₁₋₄-alkyl (meth)acrylates for use in accordance with the invention are esters of (meth)acrylic acid and straight chained or branched alcohols having 1 to 4 carbon atoms. The term "C₁₋₄-alkyl (meth)acrylates" encompasses individual (meth)acrylic esters with an alcohol of a particular length, and likewise mixtures of (meth)acrylic esters with alcohols of different lengths.

Suitable C₁₋₄-alkyl (meth)acrylates include, for example, methyl (meth)acrylate, ethyl (meth)acrylate, *n*-propyl (meth)acrylate), *iso*-propyl (meth)acrylate, *n*-butyl (meth)acrylate, *iso*-butyl (meth)acrylate and *tert*-butyl (meth)acrylate. Particularly preferred C₁₋₄-alkyl (meth)acrylates are methyl (meth)acrylate and n-butyl (meth)acrylate; methyl methacrylate and *n*-butyl methacrylate are especially preferred.

The C₁₀₋₁₅ alkyl methacrylates for use in accordance with the invention are esters of methacrylic acid and alcohols having 10 to 15 carbon atoms. The term "C₁₀₋₁₅ alkyl methacrylates" encompasses individual methacrylic esters with an alcohol of a particular length, and likewise mixtures of methacrylic esters with alcohols of different lengths.

Suitable C₁₀₋₁₅ alkyl methacrylates include, for example, decyl methacrylate, undecyl methacrylate, 5-methylundecyl methacrylate, dodecyl methacrylate, 2-methyldodecyl methacrylate, tridecyl methacrylate, 5-methyltridecyl methacrylate, tetradecyl methacrylate and/or pentadecyl methacrylate.

Particularly preferred C₁₀₋₁₅ alkyl methacrylates are methacrylic esters of a linear C₁₂₋₁₄ alcohol mixture (C₁₂₋₁₄ alkyl methacrylate).

The method according to the present invention is a free-radical polymerization. Customary free-radical polymerization is explained, inter alia, in Ullmanns's Encylopedia of Industrial Chemistry, Sixth Edition. In general, a polymerization initiator and a chain transfer agent are used for this purpose. In the process according to the present invention, the use of chain transfer agents is not necessary.

In accordance with the present invention, an initiator is added to monomer mixtures **1**, **2**, **2a** and **2b** in amounts of 0.1% to 0.5% by weight, preferably 0.1% to 0.3% by weight, based on the total amount of monomers used in the reaction. A further amount of 0.05% to 0.25% by weight, based on the total amount of monomers, of an initiator can optionally be added at the end of the reaction.

The initiator may be selected from the group consisting of azo initiators, such as azobisisobutyronitrile (AIBN), 2,2'-azobis(2-methylbutyronitrile) (AMBN) and 1,1-azobiscyclohexanecarbonitrile, and peroxy compounds such as methyl ethyl ketone peroxide, acetylacetone peroxide, dilauryl peroxide, tert-butyl per-2-ethylhexanoate, ketone peroxide, tert-butyl peroctoate, methyl isobutyl ketone peroxide, cyclohexanone peroxide, dibenzoyl peroxide, tert-butyl peroxybenzoate, tert-butyl peroxyisopropylcarbonate, 2,5-bis(2-ethylhexanoylperoxy)-2,5-dimethylhexane, tert-butyl peroxy-2-ethylhexanoate, tert-butyl peroxy-3,5,5-trimethylhexanoate, dicumyl peroxide, 1,1-bis(tert-butylperoxy)cyclohexane, 1,1-bis(tert-butylperoxy)-3,3,5-trimethylcyclohexane, cumyl hydroperoxide, tert-butyl hydroperoxide and bis(4-tert-butylcyclohexyl) peroxydicarbonate.

Preferred initiators are selected from the group consisting of 2,2'-azobis(2-methylbutyronitrile), tert-butylperoxy-2-ethylhexanoate, 1,1-di-tert-butylperoxy-3,3,5-trimethylcyclohexan, tert-butylperoxybenzoate and tert-butylperoxy-3,5,5-trimethylhexanoat. Especially preferred is tert-butylperoxy-2-ethylhexanoate.

The polymerization may be carried out at standard pressure, reduced pressure or elevated pressure. The polymerization temperature is generally in the range of 20° to 200°C, preferably 90° to 100°C.

The polymerization is carried out with a solvent. The term solvent is to be understood here in a broad sense. The solvent is selected according to the polarity of the monomers used, preference being given to using API group III oil, relatively light gas oil and/or aromatic hydrocarbons, for example toluene or xylene.

The polymerization is carried out in a suitable reaction vessel that is equipped with a stirrer and a temperature control system under nitrogen atmosphere.

The base oil to be used in the present invention comprises an oil of lubricating viscosity. Such oils include natural and synthetic oils, oil derived from hydrocracking, hydrogenation, and hydro-finishing, unrefined, refined, re-refined oils or mixtures thereof.

The base oil may also be defined as specified by the American Petroleum Institute (API) (see April 2008 version of "Appendix E-API Base Oil Interchangeability Guidelines for Passenger Car Motor Oils and Diesel Engine Oils", section 1.3 Sub-heading 1.3. "Base Stock Categories").

The API currently defines five groups of lubricant base stocks (API 1509, Annex E - API Base Oil Interchangeability Guidelines for Passenger Car Motor Oils and Diesel Engine Oils, September 2011). Groups I, II and III are mineral oils which are classified by the amount of saturates and sulphur they contain and by their viscosity indices; Group IV are polyalphaolefins; and Group V are all others, including e.g. ester oils. The table below illustrates these API classifications.

| Group | Saturates | Sulphur content | Viscosity Index (VI) |
|---|---|---|---|
| I | < 90% | > 0.03% | 80-120 |
| II | at least 90% | not more than 0.03% | 80-120 |
| III | at least 90% | not more than 0.03% | at least 120 |
| IV | All polyalphaolefins (PAOs) | | |
| V | All others not included in Groups I, II, III or IV (e.g. ester oils) | | |

The kinematic viscosity at 100°C (KV₁₀₀) of appropriate apolar base oils used to prepare an additive composition or lubricating composition in accordance with the present invention is preferably in the range of 3 mm²/s to 10 mm²/s, more preferably in the range of 4 mm²/s to 8 mm²/s, according to ASTM D445.

Further base oils which can be used in accordance with the present invention are Group II-III Fischer-Tropsch derived base oils.

Fischer-Tropsch derived base oils are known in the art. By the term "Fischer-Tropsch derived" is meant that a base oil is, or is derived from, a synthesis product of a Fischer-Tropsch process. A Fischer-Tropsch derived base oil may also be referred to as a GTL (Gas-To-Liquids) base oil. Suitable Fischer-Tropsch derived base oils that may be conveniently used as the base oil in the lubricating composition of the present invention are those as for example disclosed in EP 0 776 959, EP 0 668 342, WO 97/21788, WO 00/15736, WO 00/14188, WO 00/14187, WO 00/14183, WO 00/14179, WO 00/08115, WO 99/41332, EP 1 029 029, WO 01/18156, WO 01/57166 and WO 2013/189951.

Especially for the method according to the present invention are used base oils of API Group III, API Group V and mixtures thereof; preferred are mixtures of API Group III and API Group V base oils. As Group V base oils are preferably be used dioctylsebacate (DIOS) or Berylane.

A further object of the present invention is therefore directed to a method for preparing the polyalkyl (meth)acrylates as outlined further above, wherein
mixture **1** comprises 60% to 75% by weight of API Group III oil or mixtures thereof and 25% to 40% by weight of Group V base oil and mixtures thereof, based on the total amount of base oil used in mixture **1;** and
mixture **2** comprises 75% to 85% by weight of API Group III oil or mixtures thereof and 15% to 25% by weight of Group V base oil and mixtures thereof, based on the total amount of base oil used in mixture **2;** or
mixture **1** comprises 65% to 75% by weight of API Group III oil or mixtures thereof and 25% to 35% by weight of Group V base oil and mixtures thereof, based on the total amount of base oil used in mixture **1**;
mixture **2a** comprises 65% to 75% by weight of API Group III oil or mixtures thereof and 25% to 35% by weight of Group V base oil and mixtures thereof, based on the total amount of base oil used in mixture **2a**; and
mixture **2b** comprises 65% to 75% by weight of API Group III oil or mixtures thereof and 25% to 35% by weight of Group V base oil and mixtures thereof, based on the total amount of base oil used in mixture **2b**.

A further object of the present invention is directed to a method for the preparation of polyalkyl (meth)acrylate polymers, wherein the polyalkyl (meth)acrylate polymer consists of:
(a) 10 to 20% by weight of esters of (meth)acrylic acid and a hydroxylated hydrogenated polybutadiene;
(b1) 45% to 60% by weight of C₁₋₄ alkyl (meth)acrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N-containing monomers selected from the group consisting of N,N-dimethylaminoethyl methacrylate (DMAEMA), N-(3-(dimethylamino)propyl)methacrylamide (DMAPMAm) and N-vinylpyrrolidinone (NVP), preferably DMAEMA,

based on the total amount of the polyalkyl (meth)acrylate polymers, the method comprising the steps of:
   (i) preparing a monomer mixture **1** comprising 18 to 23% by weight of monomers (a), 45% to 52% by weight of monomers (b1), 14% to 18% by weight of monomers (b2), 9% to 11% by weight of monomers (b3) and 2.5 to 6.5% by weight of monomers (b4), based on the total amount of monomers in mixture **1**, in a base oil, the concentration of the monomers in mixture **1** being 50 to 60%; and
   (ii) adding a monomer mixture **2** comprising 6 to 11% by weight of monomers (a), 53% to 60% by weight of monomers (b1), 16 to 20% by weight of monomers (b2), 10 to 13% by weight of monomers (b3) and 3 to 7% by weight of monomers (b4), based on the total amount of monomers in mixture **2**, in a base oil, the concentration of the monomers in mixture **2** being 50 to 60%;
characterized in that monomer mixture **1** comprises 54 to 59% of the total amount of monomers used in the process and monomer mixture **2** comprises 41 to 46% of the total amount of monomers used in the process, or
   (ii) adding a monomer mixture **2a** comprising 13 to 17% by weight of monomers (a), 49% to 55% by weight of monomers (b1), 15 to 19% by weight of monomers (b2), 10 to 12% by weight of monomers (b3) and 2.5 to 7% by weight of monomers (b4), based on the total amount of monomers in mixture **2a,** in a base oil, the concentration of the monomers in mixture **2a** being 53 to 57%; and
   (iii) adding a monomer mixture **2b** comprising 0 to 1% by weight of monomers (a), 58% to 65% by weight of monomers (b1), 18 to 22% by weight of monomers (b2), 12 to 14% by weight of monomers (b3) and 3 to 8% by weight of monomers (b4), based on the total amount of monomers in mixture **2b,** in a base oil, the concentration of the monomers in mixture **2b** being 51 to 55%.
characterized in that monomer mixture **2a** comprises 23 to 27% of the total amount of monomers used in the process and monomer mixture **2b** comprises 20 to 24% of the total amount of monomers used in the process wherein
   mixture **1** comprises 60% to 75% by weight of API Group III oil or mixtures thereof and 25% to 40% by weight of Group V base oil and mixtures thereof, based on the total amount of base oil used in mixture **1**; and
   mixture **2** comprises 75% to 85% by weight of API Group III oil or mixtures thereof and 15% to 25% by weight of Group V base oil and mixtures thereof, based on the total amount of base oil used in mixture **2**; or
   mixture **1** comprises 65% to 75% by weight of API Group III oil or mixtures thereof and 25% to 35% by weight of Group V base oil and mixtures thereof, based on the total amount of base oil used in mixture **1**;
   mixture **2a** comprises 65% to 75% by weight of API Group III oil or mixtures thereof and 25% to 35% by weight of Group V base oil and mixtures thereof, based on the total amount of base oil used in mixture **2a**; and
   mixture **2b** comprises 65% to 75% by weight of API Group III oil or mixtures thereof and 25% to 35% by weight of Group V base oil and mixtures thereof, based on the total amount of base oil used in mixture **2b**.

A further first object is directed to the method as described further above, wherein the polyalkyl (meth)acrylate polymer consists of:
(a) 10 to 20% by weight of esters of (meth)acrylic acid and a hydroxylated hydrogenated polybutadiene;
(b1) 45% to 60% by weight of C₁₋₄ alkyl methacrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N,N-dimethylaminoethyl methacrylate (DMAEMA).

The content of each component (a), (b1), (b2), (b3) and (b4) is based on the total composition of the polyalkyl (meth)acrylate polymer.

In a particular embodiment, the proportions of components (a), (b1), (b2), (b3) and (b4) add up to 100% by weight.

The polymers prepared according to the method of the present invention are characterized by their contribution to low KV₄₀, HTHS₈₀ and HTHS₁₀₀ values (e.g. at a given HTHS₁₅₀ of 2.6 mPas or 2.9 mPas) of lubricating oil compositions comprising them.

The polyalkyl(meth)acrylate polymers prepared according to the method of the present invention can therefore be used in all common grades of motor oils having the viscosity characteristics defined in the document SAE J300.

The base oil to be used in the additive composition comprises an oil of lubricating viscosity as described further above.

Also disclosed is the use of an additive composition comprising at least one polyalkyl(meth)acrylate polymer prepared according to the method of the present invention and a base oil to improve the kinematic viscosity and HTHS performance of lubricating oil compositions, especially of engine oil formulations.

The invention has been illustrated by the following non-limiting examples.

### Experimental Part

### Abbreviations

- Group V oil: synthetic base oil from Total with a KV₄₀ of 2.3 cSt
- C₁₂₋₁₄ AMA: C₁₂₋₁₄-alkyl methacrylate
- CCS: cold cranking stability
- DMAEMA: dimethylaminoethyl methacrylate
- HTHS₈₀: high-temperature high-shear viscosity @80°C, measured according to CEC L-036
- HTHS₁₀₀: high-temperature high-shear viscosity @100°C, measured according to CEC L-036
- HTHS₁₅₀: high-temperature high-shear viscosity @150°C, measured according to CEC L-036
- KV: kinematic viscosity measured according to ASTM D445
- KV₄₀: kinematic viscosity @40°C, measured according to ISO 3104
- KV₁₀₀: kinematic viscosity @100°C, measured according to ISO 3104
- LMA: lauryl methacrylate;
- MM: macromonomer
- MMA: methyl methacrylate
- Mₙ: number-average molecular weight
- M_{w}: weight-average molecular weight
- NB 3020: Nexbase^{®} 3020, Group III base oil from Neste with a KV₁₀₀ of 2.2 cSt
- NB 3043: Nexbase^{®} 3043, Group III base oil from Neste with a KV₁₀₀ of 4.3 cSt
- NB 3080: Nexbase^{®} 3080, Group III base oil from Neste with a KV₁₀₀ of 8 cSt
- nBMA: *n*-butyl methacrylate
- OLOA 55501: DI Package for PCMO commercially available from Oronite
- PAO4: polyalphaolefin base oil with a KV₁₀₀ of 4 cSt
- PCMO: Passenger car motor oils
- PDI: Polydispersity index
- PPD: pour point depressant
- Sty: styrene
- VI: viscosity index, measured according to ISO 2909
- VPL^{®} 1-358: pour point depressant commercially available from Evonik
- Yubase 4+: Group III base oil from SK Lubricants with a KV₁₀₀ of 4.2 cSt

### Test methods

The polyalkyl (meth)acrylate polymers according to the present invention and the comparative examples were characterized with respect to their molecular weight and PDI.

Molecular weights were determined by size exclusion chromatography (SEC) using commercially available polymethylmethacrylate (PMMA) standards. The determination is affected by gel permeation chromatography with THF as eluent (flow rate: 1 mL/min; injected volume: 100 µl).

The additive compositions including the polyalkyl (meth)acrylate polymers according to the present invention and comparative examples were characterized with respect to their viscosity index (VI) to ASTM D 2270, kinematic viscosity at 40°C (KV₄₀) and 100°C (KV₁₀₀) to ASTM D445 and with respect to their solubility.

The lubricating oil compositions including the comb polymers according to the present invention and comparative examples were characterized with respect to kinematic viscosity at 40°C (KV₄₀) and 100°C (KV₁₀₀) to ASTM D445, the viscosity index (VI) to ASTM D 2270, high-temperature high-shear viscosity at 80°C, 100°C and 150°C to CEC L-036 and with respect to their solubility.

To show the shear stability of the lubricating oil compositions, the PSSI (Permanent Shear Stability Index) was calculated according to ASTM D 6022-01 (Standard Practice for Calculation of Permanent Shear Stability Index) based on data measured according to DIN 51381 (30 cycles of a Bosch pump).

The solubility of the additive compositions was tested in solutions of 25% polymer in Group III oil; the solubility of the lubricating oil compositions was tested in solutions of 3.75% polymer in PAO4. The solutions were analyzed photometrically after cooling down to room temperature for at least 1 day and the haze value was obtained using a Hunter LAB XE device and software. When measuring haze, the percentage of light diffusely scattered compared to the total light transmitted is reported. When the Haze level is below 5 the sample appears completely clear by eye and are considered to show very good solubility in lubricant formulations. At Haze levels between 5-10, the sample appears slightly hazy and the products are considered to show only medium solubility in lubricant formulations. At HAZE levels above 10, the sample appears obviously hazy and the products are considered to have a poor solubility in lubricant formulations.

### Synthesis of a hydroxylated hydrogenated polybutadiene

The macroalcohol prepared was a hydroxypropyl-terminated hydrogenated polybutadiene having a mean molar mass Mₙ = 4750 g/mol.

The macroalcohol was synthesized by an anionic polymerization of 1,3-butadiene with butyllithium at 20-45°C. On attainment of the desired degree of polymerization, the reaction was stopped by adding propylene oxide and lithium was removed by precipitation with methanol. Subsequently, the polymer was hydrogenated under a hydrogen atmosphere in the presence of a noble metal catalyst at up to 140°C and pressure of 200 bar. After the hydrogenation had ended, the noble metal catalyst was removed, and organic solvent was drawn off under reduced pressure. Finally, the base oil NB 3020 was used for dilution to a polymer content of 70% by weight.

The vinyl content of the macroalcohol was 61%, the hydrogenation level > 99% and the OH functionality > 98%. These values were determined by H-NMR (nuclear resonance spectroscopy).

### Synthesis of macromonomer (MM)

In a 2 L stirred apparatus equipped with saber stirrer, air inlet tube, thermocouple with controller, heating mantle, column having a random packing of 3 mm wire spirals, vapor divider, top thermometer, reflux condenser and substrate cooler, 1000 g of the above-described macroalcohol are dissolved in 450 g of methyl methacrylate (MMA) by stirring at 60°C. Added to the solution are 20 ppm of 2,2,6,6-tetramethylpiperidin-1-oxyl radical and 200 ppm of hydroquinone monomethyl ether. After heating to MMA reflux (bottom temperature about 110°C) while passing air through for stabilization, about 20 g of MMA are distilled off for azeotropic drying. After cooling to 95°C, 0.30 g of LiOCH₃ is added and the mixture is heated back to reflux. After the reaction time of about 1 hour, the top temperature has fallen to ~64°C because of methanol formation. The methanol/MMA azeotrope formed is distilled off constantly until a constant top temperature of about 100°C is established again. At this temperature, the mixture is left to react for a further hour. For further workup, the bulk of MMA is drawn off under reduced pressure. Insoluble catalyst residues are removed by pressure filtration (Seitz T1000 depth filter). The content of NB 3020 "entrained" into the copolymer syntheses described further down was taken into account accordingly.

### Synthesis of comb polymers

**Table 1: Net compositions (after reaction) of the comb polymers prepared according to the present invention.**

| **Ex. #** | **MM [%]** | **LMA [%]** | **nBMA [%]** | **Sty [%]** | **DMAEMA [%]** | **MMA [%]** |
|---|---|---|---|---|---|---|
| 1 | 13.2 | 17.4 | 51.9 | 11.2 | 6.1 | 0.2 |
| 2 | 13.5 | 17.3 | 54.3 | 11.2 | 3.5 | 0.2 |

### Example 1

### Process 1.1 (original process - comparative example):

A glass reactor equipped with a precision glass saber stirrer was initially charged with a monomer mixture **1** (= heel) having the following composition: 15% of macromonomer (70% in NB3020), 17% of LMA, 50.8% of nBMA, 11% of styrene, 6% of DMAEMA and 0.2% of MMA, based on the total amount of monomers. An oil mixture of NB3043 and Group V oil was added to achieve a concentration of monomers in oil of 55%. The resulting reaction mixture contained 45% of an oil mixture comprising 9.6% by weight of NB3020, 61.6% by weight of NB3043 and 28.8% by weight of Group V oil, based on the total amount of the oil composition.

After heating to 95°C under nitrogen, 0.15%, based on the total amount of monomers, of tert-butylperoxy-2-ethyl-hexanoate was added and the temperature maintained.

Subsequently, a monomer mixture **2** (= feed) comprising 15% of macromonomer (70% in NB3020), 17% of LMA, 50.8% of nBMA, 11% of styrene, 6% of DMAEMA and 0.2% of MMA, based on the total amount of monomers, and 0.15% by weight, based on the total amount of monomers present in the feed, of tert-butylperoxy-2-ethyl-hexanoate, was added within 3 hours with constant dosing rate. The monomer concentration of mixture **2** was 55% and the base oil was a mixture of 9.6% by weight of NB3020, 61.6% by weight of NB3043 and 28.8% of Group V oil, based on the total amount of the oil composition.

The reaction mixture obtained was further maintained at 95°C for another hour. Subsequently, another 0.2%, based on the total amount of monomers, of tert-butylperoxy-2-ethyl-hexanoate was added and the resulting reaction mixture was diluted to 40% solids with NB3043 within 3 hours. Then the reaction mixture received was again maintained at 95°C for further 2 hours and after this, another 0.1%, based on the total amount of monomers, of tert-butylperoxy-2-ethyl-hexanoate was added and the mixture was stirred at 95°C overnight. The next day, the mixture was diluted to 25% polymer with NB3043.

**Table 1.1: Composition of monomer mixtures used for the preparation of Polymer 1.1.**

| **Monomer** | **Heel** | **Feed** |
|---|---|---|
| | **[%]** | **[%]** |
| Macromonomer | 15.0 | 15.0 |
| LMA | 17.0 | 17.0 |
| nBMA | 50.8 | 50.8 |
| Styrene | 11.0 | 11.0 |
| DMAEMA | 6.0 | 6.0 |
| MMA | 0.2 | 0.2 |
| Sum | 100 | 100 |
| | | |
| Solids content | 55 | 55 |
| Oil content | 45 | 45 |
| Sum | 100 | 100 |
| | | |
| NB3020 | 9.6 | 9.6 |
| NB3043 | 61.6 | 61.6 |
| Group V oil | 28.8 | 28.8 |
| Sum | 100 | 100 |
| | | |
| Split of monomers | 50 | 50 |

This process was repeated four times using the same equipment without purification between the batches. The characteristics for the polymers prepared via the different runs are disclosed in Table 1.5 further down.

### Process 1.2 (split-feed process 1):

A glass reactor equipped with a precision glass saber stirrer was initially charged with a monomer mixture **1** (= heel) having the following composition: 20.9% of macromonomer (70% in NB3020), 15.8% of LMA, 47.3% of nBMA, 10.2% of styrene, 5.6% of DMAEMA and 0.2% of MMA, based on the total weight of the monomer composition. An oil mixture of NB3043 and Group V oil was added to achieve a concentration of monomers in oil of 55.8%. The resulting reaction mixture contained 44.2% of an oil mixture comprising 11.3% by weight of NB3020, 61% by weight of NB3043 and 27.7% by weight of Group V oil, based on the total amount of the oil composition. After heating to 95°C under nitrogen, 0.18%, based on the total amount of monomers, of tert-butylperoxy-2-ethylhexanoate was added and the temperature maintained.

Subsequently, a monomer mixture **2** (= Feed 1) comprising 15% of macromonomer (70% in NB3020), 17% of LMA, 50.8% of nBMA, 11% of styrene, 6% of DMAEMA and 0.2% of MMA, based on the total amount of monomers, and 0.18% by weight, based on the total amount of monomers present in the feed, of tert-butylperoxy-2-ethyl-hexanoate, in an oil mixture of NB3043 and Group V oil was added within 1.5 hours with constant dosing rate. Monomer mixture **2** contained 55% of monomers and 45% of an oil mixture comprising 7.9% by weight of NB3020, 63.3% by weight of NB3043 and 28.8% by weight of Group V oil, based on the total amount of the oil composition.

Subsequently, a monomer mixture **3** (= Feed 2) comprising 20% of LMA, 59.8% of nBMA, 12.9% of styrene, 7.1% of DMAEMA and 0.2% of MMA, based on the total amount of monomers, and 0.18% by weight, based on the total amount of monomers present in the feed, of tert-butylperoxy-2-ethylhexanoate, in an oil mixture of NB3043 and Group V oil was added within 1.5 hours with constant dosing rate. Monomer mixture **3** contained 53% of monomers and 47% of an oil mixture comprising 68.8% by weight of NB3043 and 31.2% by weight of Group V oil, based on the total amount of the oil composition. After that, the reaction was maintained at 95°C for another hour.

Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 h and after this another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 1.2: Composition of monomer mixtures used for the preparation of Polymer 1.2.**

| **Monomer** | **Heel** | **Feed 1** | **Feed 2** |
|---|---|---|---|
| | **[%]** | **[%]** | **[%]** |
| Macromonomer | 20.9 | 15.0 | 0 |
| LMA | 15.8 | 17.0 | 20.0 |
| nBMA | 47.3 | 50.8 | 59.8 |
| Styrene | 10.2 | 11.0 | 12.9 |
| DMAEMA | 5.6 | 6.0 | 7.1 |
| MMA | 0.2 | 0.2 | 0.2 |
| Sum | 100 | 100 | 100 |
| | | | |
| Solids content | 55.8 | 55.0 | 53.0 |
| Oil content | 44.2 | 45.0 | 47.0 |
| Sum | 100 | 100 | 100 |
| | | | |
| NB3020 | 11.3 | 7.9 | 0 |
| NB3043 | 61.0 | 63.3 | 68.8 |
| Group V oil | 27.7 | 28.8 | 31.2 |
| Sum | 100 | 100 | 100 |
| | | | |
| Split of monomers | 53 | 25 | 22 |

This process was also repeated four times using the same equipment without purification between the batches. The characteristics for the polymers prepared via the different runs are disclosed in Table 1.5 further down.

### Process 1.3 (split-feed process 2):

A glass reactor equipped with a precision glass saber stirrer was initially charged with a monomer mixture **1** (= Heel) having the following composition: 20.9% of macromonomer (70% in NB3020), 15.8% of LMA, 47.2% of nBMA, 10.2% of styrene, 5.6% of DMAEMA and 0.3% of MMA, based on the total weight of the monomer composition. An oil mixture of NB3043 and Group V oil was added to achieve a concentration of monomers in oil of 52.6%. The resulting reaction mixture contained 47.4% of an oil mixture comprising 10% by weight of NB3020, 53.5% by weight of NB3043 and 36.5% by weight of Group V oil, based on the total amount of the oil composition. After heating to 95°C under nitrogen, 0.15%, based on the total amount of monomers, of tert-butylperoxy-2-ethylhexanoate was added and the temperature maintained.

Subsequently, a monomer mixture **2** (= Feed) comprising 8.1% of macromonomer (70% in NB3020), 18.4% of LMA, 55% of nBMA, 11.9% of styrene, 6.5% of DMAEMA and 0.1% of MMA, based on the total amount of monomers, and 0.15%, based on the total amount of monomers, of tert-butylperoxy-2-ethyl-hexanoate in an oil mixture of NB3043 and Group V oil was added within 3 hours with constant dosing rate. Monomer mixture **2** contained 58% of monomers and 42% of an oil mixture comprising 4.8% by weight of NB3020, 77.6% by weight of NB3043 and 17.6% by weight of Group V oil, based on the total amount of the oil composition. The resulting reaction mixture was then maintained at 95°C for another hour.

Subsequently, the reaction mixture was diluted to 40% solids with NB3043 and 0.2%, based on the total amount of monomers, of tert-butylperoxy-2-ethyl-hexanoate within one hour. Then the reaction was again maintained at 95°C for another hour and after this, another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 1.3: Composition of monomer mixtures used for the preparation of Polymer 1.3.**

| **Monomer** | **Heel** | **Feed** |
|---|---|---|
| | **[%]** | **[%]** |
| Macromonomer | 20.9 | 8.1 |
| LMA | 15.8 | 18.4 |
| nBMA | 47.2 | 55.0 |
| Styrene | 10.2 | 11.9 |
| DMAEMA | 5.6 | 6.5 |
| MMA | 0.3 | 0.1 |
| Sum | 100 | 100 |
| | | |
| Solids content | 52.6 | 58.0 |
| Oil content | 47.4 | 42 |
| Sum | 100 | 100 |
| | | |
| NB3020 | 10.0 | 4.8 |
| NB3043 | 53.5 | 77.6 |
| Group V oil | 36.5 | 17.6 |
| Sum | 100 | 100 |
| | | |
| Split of monomers | 56.2 | 43.8 |

### Process 1.4 (split-feed process 3):

An apparatus with 4-neck flask and precision glass saber stirrer was initially charged with a monomer mixture **1** (= Heel) having the following composition: 19.8% of macromonomer (70% in NB3020), 16% of LMA, 47.9% of nBMA, 10.4% of styrene, 5.6% of DMAEMA and 0.3% of MMA, based on the total weight of the monomer composition. An oil mixture of NB3043 and Group V oil was added to achieve a concentration of monomers in oil of 55%. The resulting reaction mixture contained an oil mixture comprising 10.4% by weight of NB3020, 60.8% by weight of NB3043 and 28.8% by weight of Group V oil, based on the total amount of the base oil composition. After heating to 95°C under nitrogen, 0.18%, based on the total amount of monomers, of tert-butylperoxy-2-ethyl-hexanoate was added and the temperature maintained.

Subsequently, a monomer mixture **2** (= Feed) comprising 8.7% of macromonomer (70% in NB3020), 18.3% of LMA, 54.6% of nBMA, 11.8% of styrene, 6.5% of DMAEMA and 0.1% of MMA, based on the total amount of monomers, and 0.18%, based on the total amount of monomers, of tert-butylperoxy-2-ethyl-hexanoate was added within 3 hours with constant dosing rate. Monomer mixture **2** contained 55% of monomers and 45% of an oil mixture comprising 4.5% by weight of NB3020, 76.1% by weight of NB3043 and 19.4% by weight of Group V oil, based on the total amount of the oil composition. The resulting reaction mixture was then maintained at 95°C for another hour.

Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 hours and after this another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 1.4: Composition of monomer mixtures used for the preparation of Polymer 1.4.**

| **Monomer** | **Heel** | **Feed** |
|---|---|---|
| | **[%]** | **[%]** |
| Macromonomer | 19.8 | 8.7 |
| LMA | 16.0 | 18.3 |
| nBMA | 47.9 | 54.6 |
| Styrene | 10.4 | 11.8 |
| DMAEMA | 5.6 | 6.5 |
| MMA | 0.3 | 0.1 |
| Sum | 100 | 100 |
| | | |
| Solids content | 55 | 55 |
| Oil content | 45 | 45 |
| Sum | 100 | 100 |
| | | |
| NB3020 | 10.4 | 4.5 |
| NB3043 | 60.8 | 76.1 |
| Group V oil | 28.8 | 19.4 |
| Sum | 100 | 100 |
| | | |
| Split of monomers | 56.8 | 43.2 |

The following Table 1.5 shows the molecular weights, polydispersity and HAZE values of Polymers 1.

**Table 1.5: Characteristics of Polymers 1.**

| **Polymer** | **Run** | **Content** | **Mₙ** | **M_{W}** | **D** | **Haze*⁾** |
|---|---|---|---|---|---|---|
| | **#** | **[%]** | **[g/mol]** | **[g/mol]** | | |
| 1.1 (CE) | 1 | 25 | 148,000 | 547,000 | 3.7 | 2.3 |
| | 2 | 25 | 144,000 | 524,000 | 3.7 | 3.1 |
| | 3 | 25 | 146,000 | 528,000 | 3.6 | 9.8 |
| | 4 | 25 | 125,000 | 513,000 | 4.1 | 14.0 |
| 1.2 | 1 | 25 | 137,000 | 534,000 | 3.9 | 2.8 |
| | 2 | 25 | 131,000 | 518,000 | 4.0 | 3.1 |
| | 3 | 25 | 139,000 | 514,000 | 3.7 | 1.2 |
| | 4 | 25 | 160,000 | 532,000 | 3.3 | 4.1 |
| 1.3 | | 25 | 137,000 | 582,000 | 4.3 | 1.0 |
| 1.4 | | 25 | 153,000 | 550,000 | 3.6 | 1.4 |

| | | | | | | |
|---|---|---|---|---|---|---|
| *⁾...Determined in product (25% polymer in oil). CE = comparative example | | | | | | |

It can be seen that using the old process 1.1 led to an increase of haziness of the pure product from batch 1 to batch 4 during the manufacturing process. Where run 1 and run 2 still showed good haze values of below 5, i.e. the solutions appeared clean, runs 3 and 4 showed haze values of 10 and 14, respectively and appeared hazy. As the haze value is an indicator for the solubility of the polymers in lubricants and especially engine oil formulations, the polymers retrieved with runs 3 and 4 would not be soluble.

When using the split-feed process 1.2, the haze values of all products from the 4 runs were well below 5. Especially, the haze value of the polymer of the 4^{th} batch was reduced from 14 (comparative example 1.1) to 4.1. That ensures the applicability of the polymers in engine oil formulations.

Consequently, the reduction in haze leads to a significant efficiency gain in the production. For example, a kettle needs to be cleaned as soon as the product haze raises to 10. That means that for the split-feed processes 1.2, 1.3 and 1.4 at least four batches can be produced in a row before cleaning the kettle. This is not possible for the process 1.1, where the kettle would have to be cleaned latest after the third batch.

Using the split-feed process according to the present invention does therefore lead to an increased production output.

Additionally, the method according to the present invention allows the upscaled production of Polymers 1 in a plant.

In the following Table 1.6, the HAZE values and viscosities of 3.75% Polymers 1 in oil are disclosed.

**Table 1.6: Viscosities of 3.75% Polymers 1 in a Group III base oil mixture (NB 3043 and NB 3080 from Neste) with KV₁₀₀ of 4.9 cSt.**

| **Polymer** | **Run #** | **Content [%]** | **KV₁₀₀ [mm²/s]** | **KV₄₀ [mm²/s]** | **VI** | **HAZE*⁾** |
|---|---|---|---|---|---|---|
| 1.1 (CE) | 1 | 3.75 | 7.65 | 29.21 | 260 | 2.5 |
| | 2 | 3.75 | 7.61 | 28.60 | 255 | 3.6 |
| | 3 | 3.75 | 7.61 | 28.60 | 255 | 4.5 |
| | 4 | 3.75 | 7.61 | 28.57 | 256 | 6.9 |
| 1.2 | 1 | 3.75 | 7.68 | 28.51 | 260 | 2.1 |
| | 2 | 3.75 | 7.66 | 28.52 | 259 | 2.9 |
| | 3 | 3.75 | 7.62 | 28.51 | 257 | 2.7 |
| | 4 | 3.75 | 7.70 | 28.54 | 260 | 1.3 |
| 1.3 | | 3.75 | 7.59 | 28.35 | 257 | 1.4 |
| 1.4 | | 3.75 | 7.71 | 28.70 | 259 | 1.7 |

| | | | | | | |
|---|---|---|---|---|---|---|
| *⁾...Determined from a composition of 3.75% polymer in PAO4. CE = comparative example | | | | | | |

It can be seen that the sample comprising Polymer 1.1 that was prepared following the known process appears to be slightly hazy, whereas Polymers 1.2, 1.3 and 1.4 prepared according to the method of the present invention appear clear with haze levels well below 5.

Especially, when comparing Polymer 1.1 of run 4 with Polymer 1.2 of run 4 it can be seen that using the novel split-feed process of the present invention instead of a common process leads to an improved solubility of the product in oil, reflected in a haze value of 1.3 (Polymer 1.2, run 4) instead of 6.9 (Polymer 1.1, run 4).

### Example 2

### Process 2.1 (original process - comparative example):

A glass reactor equipped with a precision glass saber stirrer was initially charged with a monomer mixture **1** (= heel) having the following composition: 15% of macromonomer (70% in NB3020), 17% of LMA, 53% of nBMA, 11% of styrene and 3% of DMAEMA. An oil mixture of NB3043 and Group V oil was added to achieve a concentration of monomers in oil of 55%. The resulting reaction mixture contained 45% of an oil mixture comprising 7.9% by weight of NB3020, 63.3% by weight of NB3043 and 28.8% by weight of Group V oil, based on the total amount of the oil composition.

After heating to 95°C under nitrogen, 0.18%, based on the total amount of monomers, of tert-butylperoxy-2-ethyl-hexanoate was added and the temperature maintained.

Subsequently, a monomer mixture **2** (= feed) comprising 15% of macromonomer (70% in NB3020), 17% of LMA, 53% of nBMA, 11% of styrene and 3% of DMAEMA, based on the total amount of monomers, and 0.18%, based on the total amount of monomers, of tert-butylperoxy-2-ethylhexanoate in an oil mixture of NB3043 and Group V oil was added within 3 hours with constant dosing rate. Monomer mixture **2** contained 55% of monomers and 45% of an oil mixture comprising 7.9% by weight of NB3020, 63.3% by weight of NB3043 and 28.8% by weight of Group V oil, based on the total amount of the oil composition.

The reaction was further maintained at 95°C for another hours. Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 hours and after this, another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 2.1: Composition of monomer mixtures used for the preparation of Polymer 2.1.**

| **Monomer** | **Heel** | **Feed** |
|---|---|---|
| | **[%]** | **[%]** |
| Macromonomer | 15.0 | 15.0 |
| LMA | 17.0 | 17.0 |
| nBMA | 53.4 | 53.4 |
| Styrene | 11.0 | 11.0 |
| DMAEMA | 3.4 | 3.4 |
| MMA | 0.2 | 0.2 |
| Sum | 100 | 100 |
| | | |
| Solids content | 55 | 55 |
| Oil content | 45 | 45 |
| Sum | 100 | 100 |
| | | |
| NB3020 | 7.9 | 7.9 |
| NB3042 | 63.3 | 63.3 |
| Group V oil | 28.8 | 28.8 |
| Sum | 100 | 100 |
| | | |
| Split of monomers | 50 | 50 |

In this case, the process was not repeated four times using the same equipment. From process 1.1 it can be seen that the haze values raised from 2.3 (process 1.1, run 1) to 3.1 (process 1.1, run 2) and 9.8 (process 1.1, run 3). This raise was observed for 6.1% of the polar monomer DMAEMA (corresponds to component (b4)). It can be expected that the raise between the runs would be similar for process 2.1 as well.

### Process 2.2 (split-feed process 1):

A glass reactor equipped with a precision glass saber stirrer was initially charged with a monomer mixture **1** (= heel) having the following composition: 20.9% of macromonomer (70% in NB3020), 15.8% of LMA, 49.7% of nBMA, 10.2% of styrene, 3.2% of DMAEMA and 0.2% of MMA, based on the total weight of the monomer composition. An oil mixture of NB3043 and Group V oil was added to achieve a concentration of monomers in oil of 55.8%. The resulting reaction mixture contained 44.2% of an oil mixture comprising 11.3% by weight of NB3020, 61% by weight of NB3043 and 27.2% by weight of Group V oil, based on the total amount of the oil composition. After heating to 95°C under nitrogen, 0.18%, based on the total amount of monomers, of tert-butylperoxy-2-ethylhexanoate was added and the temperature maintained.

Subsequently, a monomer mixture **2** (= feed 1) comprising 15% of macromonomer (70% in NB3020), 17% of LMA, 53.4% of nBMA, 11% of styrene, 3.4% of DMAEMA and 0.2% of MMA, based on the total amount of monomers, and 0.18%, based on the total amount of monomers, of tert-butylperoxy-2-ethyl-hexanoate in an oil mixture comprising NB3043 and Group V oil was added within 1.5 hours with constant dosing rate. Monomer mixture **2** contained 55% of monomers and 45% of an oil mixture comprising 7.9% by weight of NB3020, 36.3% by weight of NB3043 and 28.8% by weight of Group V oil, based on the total amount of the oil composition.

Subsequently, a monomer mixture **3** (= feed 2) comprising 20% of LMA, 62.8% of nBMA, 12.9% of styrene, 4.0% of DMAEMA and 0.2% of MMA, based on the total amount of monomers, and 0.18% by weight, based on the total amount of monomers present in the feed, of tert-butylperoxy-2-ethylhexanoate in an oil mixture comprising NB3043 and Group V oil was added within 1.5 hours with constant dosing rate. Monomer mixture **3** contained 53% of monomers and 47% of an oil mixture comprising 68.8% by weight of NB3043 and 31.2% by weight of Group V oil, based on the total amount of the oil composition. After that, the reaction was maintained at 95°C for another hour. Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 h and after this another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 2.2: Composition of monomer mixtures used for the preparation of Polymer 2.2.**

| **Monomer** | **Heel** | **Feed 1** | **Feed 2** |
|---|---|---|---|
| | **[%]** | **[%]** | **[%]** |
| Macromonomer | 20.9 | 15.0 | 0 |
| LMA | 15.8 | 17.0 | 20.0 |
| nBMA | 49.7 | 53.4 | 62.8 |
| Styrene | 10.2 | 11.0 | 12.9 |
| DMAEMA | 3.2 | 3.4 | 4.0 |
| MMA | 0.2 | 0.2 | 0.2 |
| Sum | 100 | 100 | 100 |
| | | | |
| Solids content | 55.8 | 55.0 | 53.0 |
| Oil content | 44.2% | 45% | 47% |
| Sum | 100 | 100 | 100 |
| | | | |
| NB3020 | 11.3 | 7.9 | 0 |
| NB3043 | 61.0 | 36.3 | 68.8 |
| Group V oil | 27.7 | 28.8 | 31.2 |
| Sum | 100 | 100 | 100 |
| | | | |
| Split of monomers | 53 | 25 | 22 |

### Process 2.3 (split-feed process 2):

A glass reactor equipped with a precision glass saber stirrer was initially charged with a monomer mixture **1** (= heel) having the following composition: 20.0% of macromonomer (70% in NB3020), 15.8% of LMA, 49.6% of nBMA, 10.2% of styrene, 3.2% of DMAEMA and 0.3% of MMA, based on the total weight of the monomer composition. An oil mixture of NB3043 and Group V oil was added to achieve a concentration of monomers in oil of 52.6%. The resulting reaction mixture contained an oil mixture comprising 10% by weight of NB3020, 53.5% by weight of NB3043 and 36.5% by weight of Group V oil, based on the total amount of the oil composition. After heating to 95°C under nitrogen, 0.15%, based on the total amount of monomers, of tert-butylperoxy-2-ethyl-hexanoate was added and the temperature maintained.

Subsequently, a monomer mixture **2** (= feed) comprising 8.1% of macromonomer (70% in NB3020), 18.4% of LMA, 57.8% of nBMA, 11.9% of styrene, 3.7% of DMAEMA and 0.1% of MMA, based on the total amount of monomers, and 0.15%, based on the total amount of monomers, of tert-butylperoxy-2-ethyl-hexanoate in an oil mixture comprising NB3043 and Group V oil was added within 3 hours with constant dosing rate. Monomer mixture **2** contained 58% of monomers and 42% of an oil mixture comprising 4.8% by weight of NB3020, 77.6% by weight of NB3043 and 17.6% by weight of Group V oil, based on the total amount of the oil composition. The resulting reaction mixture was then maintained at 95°C for another hour.

Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 hours and after this another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 2.3: Composition of monomer mixtures used for the preparation of Polymer 2.3.**

| **Monomer** | **Heel** | **Feed** |
|---|---|---|
| | **[%]** | **[%]** |
| Macromonomer | 20.9 | 8.1 |
| LMA | 15.8 | 18.4 |
| nBMA | 49.6 | 57.8 |
| Styrene | 10.2 | 11.9 |
| DMAEMA | 3.2 | 3.7 |
| MMA | 0.3 | 0.1 |
| Sum | 100 | 100 |
| | | |
| Solids content | 52.6 | 58.0 |
| Oil content | 47.4 | 42.0 |
| Sum | 100 | 100 |
| | | |
| NB3020 | 10.0 | 4.8 |
| NB3043 | 53.3 | 77.6 |
| Group V oil | 36.5 | 17.6 |
| Sum | 100 | 100 |
| | | |
| Split of monomers | 56.2 | 43.8 |

This process was repeated four times using the same equipment without purification between the batches. The characteristics for the polymers prepared via the different runs are disclosed in Table 2.5 further down.

### Process 2.4 (split-feed process 3):

A glass reactor equipped with a precision glass saber stirrer was initially charged with a monomer mixture **1** (= heel) having the following composition: 19.8% of macromonomer (70% in NB3020), 16.0% of LMA, 50.3% of nBMA, 10.4% of styrene, 3.2% of DMAEMA and 0.3% of MMA, based on the total weight of the monomer composition. An oil mixture of NB3043 and Group V oil was added to achieve a concentration of monomers in oil of 60%. The resulting reaction mixture contained an oil mixture comprising 12.7% by weight of NB3020, 58.7% by weight of NB3043 and 28.6% by weight of Group V oil, based on the total amount of the oil composition. After heating to 95°C under nitrogen, 0.18%, based on the total amount of monomers, of tert-butylperoxy-2-ethyl-hexanoate was added and the temperature maintained.

Subsequently, a monomer mixture **2** (= feed) comprising 8.7% of macromonomer (70% in NB3020), 18.3% of LMA, 57.4% of nBMA, 11.8% of styrene, 3.7% of DMAEMA and 0.1% of MMA, based on the total amount of monomers, and 0.18%, based on the total amount of monomers, of tert-butylperoxy-2-ethyl-hexanoate in an oil mixture comprising NB3043 and Group V oil was added within 3 hours with constant dosing rate. Monomer mixture **2** contained 60% of monomers and 40% of an oil mixture comprising 5.6% by weight of NB3020, 75% by weight of NB3043 and 19.4% by weight of Group V oil, based on the total amount of the oil composition. The resulting reaction mixture was then maintained at 95°C for another hour.

Subsequently, the reaction mixture was diluted to 40% solids with NB3043 and 0.2%, based on the total amount of monomers, of tert-butylperoxy-2-ethyl-hexanoate within 3 hours. Then the reaction was again maintained at 95°C for another 2 hours and after this another 0.1%, based on the total amount of monomers, of tert-butylperoxy-2-ethyl-hexanoate was added and the mixture was stirred at 95°C overnight. The next day, the mixture was diluted to 25% solids with NB3043.

**Table 2.4: Composition of monomer mixtures used for the preparation of Polymer 2.4.**

| **Monomer** | **Heel** | **Feed** |
|---|---|---|
| | **[%]** | **[%]** |
| Macromonomer | 19.8 | 8.7 |
| LMA | 16.0 | 18.3 |
| nBMA | 50.3 | 57.4 |
| Styrene | 10.4 | 11.8 |
| DMAEMA | 3.2 | 3.7 |
| MMA | 0.3 | 0.1 |
| Sum | 100 | 100 |
| | | |
| Solids content | 60 | 60 |
| Oil content | 40 | 40 |
| Sum | 100 | 100 |
| | | |
| NB3020 | 12.7 | 5.6 |
| NB3043 | 58.7 | 75.0 |
| Group V oil | 28.6 | 19.4 |
| Sum | 100 | 100 |
| | | |
| Split of monomers | 56.8 | 43.2 |

The following Table 2.5 shows the molecular weights, polydispersity and HAZE values of Polymers 2.

**Table 2.5: Characteristics of Polymers 2.**

| **Polymer** | **Run** | **Content** | **Mₙ** | **M_{W}** | **D** | **HAZE*⁾** |
|---|---|---|---|---|---|---|
| | **#** | **[%]** | **[g/mol]** | **[g/mol]** | | |
| 2.1 (CE) | 1 | 25 | 144,000 | 494,000 | 3.4 | 4.2 |
| 2.2 | 1 | 25 | 165,000 | 513,000 | 3.1 | 0 |
| 2.3 | 1 | 25 | 149,000 | 478,000 | 3.2 | 2.0 |
| | 2 | 25 | 134,000 | 470,000 | 3.5 | 2.7 |
| | 3 | 25 | 127,000 | 485,000 | 3.8 | 4.0 |
| | 4 | 25 | 149,000 | 488,000 | 3.3 | 7.1 |
| 2.4 | 1 | 25 | 142,000 | 524,000 | 3.7 | 4.2 |

| | | | | | | |
|---|---|---|---|---|---|---|
| *⁾...Determined in product. CE = comparative example | | | | | | |

It can be seen that the HAZE values of the polymers retrieved out of the different syntheses are well below 5. That means that the polymers are soluble in oil, i.e. the solution appears clear.

In the following Table 2.6, the HAZE values and viscosities of 3.75% Polymers 2 in oil are disclosed.

**Table 2.6: Viscosities of 3.75% Polymers 2 in a Group III base oil mixture (NB 3043 and NB 3080 from Neste) with KV₁₀₀ of 4.9 cSt.**

| **Polymer** | **Run** | **Content** | **KV₁₀₀** | **KV₄₀** | **VI** | **HAZE*⁾** |
|---|---|---|---|---|---|---|
| | **#** | **[%]** | **[mm²/s]** | **[mm²/s]** | | |
| 2.1 (CE) | 1 | 3.75 | 7.81 | 28.76 | 264 | 0.6 |
| 2.2 | | 3.75 | 7.95 | 28.53 | 274 | 0.3 |
| 2.3 | 1 | 3.75 | 7.85 | 28.69 | 267 | 1.9 |
| | 2 | 3.75 | 7.77 | 28.79 | 267 | 2.3 |
| | 3 | 3.75 | 7.85 | 28.77 | 267 | 1.6 |
| | 4 | 3.75 | 7.93 | 28.80 | 267 | 4.6 |
| 2.4 | | 3.75 | 8.29 | 29.34 | 281 | |

| | | | | | | |
|---|---|---|---|---|---|---|
| *⁾...Determined from a composition of polymer in PAO4. CE = comparative example | | | | | | |

The problem usually arising from using known processes is that the reaction mixtures used to prepare commonly known polyalkyl (meth)acrylates contain monomers with different reactivities leading to polymers with an inhomogenous distribution of the apolar and polar monomers. If one monomer is more reactive than another second monomer, this monomer will be copolymerized in a higher amount in the beginning of the monomer feed leading to polymer compositions with increased amounts of this monomer at the beginning, while the second monomer will be enriched in the polymers formed during a later time in the feed process. The final product then contains a mixture of all the different fractions of the polymer compositions formed during the whole process, from more polar to less polar fractions as compared to the average polymer composition. Typically, these are only very small deviations. But for polymerizations where macromonomers are used and especially in combination with dispersant monomers like DMAEMA the deviations are extremely large.

The following Table 3 shows the polymerization kinetics of Polymer 1.1 during the original process 1.1. The composition of generated and accumulated polymer is shown over the time.

**Table 3: Composition of generated and accumulated Polymer 1.1 over time.**

| **Monomer [%]** | **Time [min]** | | | | | | | | **Variation** |
|---|---|---|---|---|---|---|---|---|---|
| | 0 | 30 | 60 | 120 | 180 | 240 | 540 | 700 | |
| MM | 0 | 3.5 | 18.6 | 12.4 | 14.5 | 11.2 | 22.2 | 14.1 | 3-23 |
| LMA | 0 | 17.7 | 21.3 | 14.8 | 18.4 | 13.5 | 18.9 | 17.6 | 13-22 |
| nBMA | 0 | 52.7 | 37.2 | 55.9 | 49.1 | 59.3 | 47.2 | 64.6 | 37-65 |
| Sty | 0 | 15.1 | 15.7 | 12.3 | 12.4 | 10.4 | 6.3 | 0 | 0-16 |
| DMAEMA | 0 | 11.2 | 6.7 | 4.5 | 5.3 | 5.3 | 5.2 | 4.0 | 4-12 |
| MMA | 0 | -0.2 | 0.5 | 0.2 | 0.3 | 0.3 | 0.2 | -0.3 | 0-0.5 |
| generated amount of polymer | 0 | 16.0 | 8.4 | 22.0 | 17.4 | 14.7 | 20.6 | 1.0 | |
| accumulated amount of polymer | 0 | 16.0 | 24.3 | 46.3 | 63.7 | 78.4 | 99.0 | 100 | |

In Table 3, in each column the composition of the polymer produced in this time interval and the percentage of this polymer fraction in the final mixture (= amount generated in each time interval) can be found. The amounts of different monomers are determined by measuring the residual monomer contents of each sample.

From the data presented in Table 3, it can be seen how inhomogeneous the conversion of the varying monomers is over the polymerization time and that the composition differs significantly from one time interval to the other. Especially, the content of macromonomer (MM) varies between 3 and 23% and the content of butyl methacrylate (BMA) varies between 37 and 65%.

The following Table 4 shows the polymerization kinetics of Polymer 1.2 having the same total composition as Polymer 1.1 but was produced using the "split-feed" process 1.2. The composition of generated and accumulated polymer is shown over the time.

The compositional differences of the product fractions prepared via the different processes becomes visible when both sets of kinetics data are compared.

**Table 4: Composition of generated and accumulated Polymer 1.2 over time.**

| **Monomer [%]** | **Time [min]** | | | | | | | | | **Variation** |
|---|---|---|---|---|---|---|---|---|---|---|
| | 0 | 30 | 60 | 90 | 120 | 180 | 240 | 420 | 700 | |
| MM | 0 | 19.2 | 5.8 | 17.3 | 13.1 | 12.3 | 8.9 | 16.6 | 20.7 | 5-21 |
| LMA | 0 | 13.3 | 21.9 | 9.3 | 19.6 | 18.8 | 14.9 | 19.2 | 18.2 | 9-22 |
| nBMA | 0 | 47.7 | 51.3 | 51.6 | 50.6 | 49.3 | 58.9 | 51.2 | 52.6 | 47-59 |
| Sty | 0 | 14.5 | 13.3 | 15.0 | 10.6 | 12.7 | 11.1 | 6.8 | 3.5 | 3-15 |
| DMAEMA | 0 | 5.3 | 7.5 | 6.9 | 5.7 | 6.6 | 5.9 | 5.9 | 4.8 | 4-8 |
| MMA | 0 | 0 | 0.2 | -0.1 | 0.4 | 0.3 | 0.3 | 0.2 | 0.1 | 0-0.4 |
| generated amount of polymer | 0 | 15.7 | 10.2 | 9.1 | 14.1 | 14.9 | 15.1 | 16.2 | 4.7 | |
| accumulated amount of polymer | 0 | 15.7 | 25.8 | 34.9 | 49.0 | 63.9 | 79.1 | 95.3 | 100 | |

In Table 4, in each column the composition of the polymer produced in this time interval and the percentage of this polymer fraction in the final mixture (= amount generated in each time interval) can be found. It can be seen that using a split-feed process leads to a more homogeneous conversion of the varying monomers over the polymerization time and that the composition differs less from one time interval to the other.

The ratio between polar (nBMA, Sty, DMAEMA) and unpolar (>=C12) alkyl methacrylates in the composition of the different polymer fractions was calculated. Corresponding values are presented in the following Tables 5 (for Process 1.1) and 6 (for Process 1.2).

**Table 5: Original process 1.1.**

| **Time** | **Conversion of MM+LMA** | **Conversion of nBMA+Sty+ DMAEMA+MMA** | **Ratio polar/unpolar monomers** | **Conversion per fraction** |
|---|---|---|---|---|
| **[min]** | **[%]** | **[%]** | | **[%]** |
| 0 | 0 | 0 | 0 | 0 |
| 30 | 21.2 | 78.8 | 3.7 | 16.0 |
| 60 | 39.8 | 60.2 | 1.5 | 8.4 |
| 120 | 27.2 | 72.8 | **2.7** | **22.0** |
| 180 | 32.8 | 67.2 | **2.0** | **17.4** |
| 240 | 24.7 | 75.3 | 3.0 | 14.7 |
| 540 | 41.1 | 58.9 | 1.4 | 20.6 |
| 700 | 31.7 | 68.3 | **2.2** | **1.0** |
| Average | **27.3** | **60.2** | | |
| Summarized fractions fulfilling the requirement | | | **2.2 +/- 0.66** | **40.4** |

**Table 6: Split-feed process 1.2.**

| **Time** | **Conversion of MM+LMA** | **Conversion of nBMA+Sty+ DMAEMA+MMA** | **Ratio polar/unpolar monomers** | **Conversion per fraction** |
|---|---|---|---|---|
| **[min]** | **[%]** | **[%]** | | **[%]** |
| 0 | 0 | 0 | 0 | 0 |
| 30 | 32.4 | 67.6 | **2.1** | **15.3** |
| 60 | 27.7 | 72.3 | **2.6** | **10.0** |
| 90 | 26.7 | 73.3 | **2.8** | **8.9** |
| 120 | 32.7 | 67.3 | **2.1** | **14.0** |
| 180 | 31.0 | 69.0 | **2.2** | **10.2** |
| 240 | 23.8 | 76.2 | 3.2 | 19.9 |
| 420 | 35.8 | 64.2 | **1.8** | **16.6** |
| 700 | 39.0 | 61.0 | 1.6 | 5.2 |
| Average | 31.1 | 68.9 | | |
| Summarized fractions fulfilling the requirement | | | **2.2 +/- 0.66** | **80.1** |

This ratio can be used as an estimate for the overall polarity of the polymer in each fraction prepared in the respective time intervals and is therefore used as an estimate for the solubility/HAZE of the polymer in this fraction. Comparing the polarity ratios of the two process variants leads to the result that for the original process larger deviations from the average polarity ratio of the polymer exist.

In contrast, only small deviations from the average polarity ratio were found for the new split feed processes. For example, for the original process 1.1, 59.6% of the formed polymers deviate more than 30% from the average polarity ratio while for the new split feed process 1.2 only 19.9% of the formed polymers deviate more than 30% from the average polarity ratio. This means that for the original process only about 40% of the produced product lies in the window of a composition with less than 30% deviation while for the new split feed process more than 80% of the produced polymer has a composition with less than 30% deviation. Together with the Haze values of the product and the production in oil solution this supports the concept that a reduction of the most polar species can help to improve product properties like its solubility or producibility.

The kinetics can be calculated via the residual monomer content(s).

### Evaluation of VI improvers in formulations

To demonstrate the effect of the polyalkyl(methacrylate) polymers according to the present invention on the KV₄₀ and HTHS₁₀₀ performance of lubricating oil compositions different formulation examples were prepared and the corresponding values are measured. Formulations with Yubase 4+ as base oil were prepared by using formulation targets 0W30 according to SAE J300; i.e. it was formulated on an HTHS₁₅₀ target of 2.9 mPas by adding the polymers prepared according to the present invention. The resulting polymer content was typically between 3 and 3.5% by weight. Characteristic EO formulation properties (KV₄₀, KV₁₀₀, HTHS₁₀₀, HTHS₈₀) were measured and are summarized in Table 7 below.

**Table 7: 0W30 engine oil formulations A of Polymers 1 and 2 with DI package in Yubase 4+ as base oil, adjusted to HTHS₁₅₀ = 2.9 mPas.**

| **Composition** | **A1** | **A2** |
|---|---|---|
| | | |
| Polymer 1.4 [wt%] | 12.9 | -- |
| | | |
| Solids content [%] | 3.2 | -- |
| Polymer 2.4 [wt%] | -- | 12.3 |
| Solids content [%] | -- | 3.1 |
| PPD (VPL 1-358) [wt%] | 0.2 | 0.2 |
| OLOA 55501 [wt%] | 8.9 | 8.9 |
| Yubase 4+ [wt%] | 78.0 | 78.6 |
| Sum | 100 | 100 |
| | | |

| **Test method** | | |
|---|---|---|
| | | |
| KV₄₀ [mm²/s] | 29.74 | 29.18 |
| KV₁₀₀ [mm²/s] | 8.41 | 8.21 |
| VI | 282 | 279 |
| HTHTS₁₅₀ [mPas] | 2.93 | 2.93 |
| HTHS₁₀₀ [mPas] | 5.37 | 5.28 |
| HTHS₈₀ [mPas] | 7.76 | 7.62 |
| CCS @-35°C | 3807 | 3752 |
| Shear loss @KV₁₀₀ after Bosch Injector 30 cycles [%] | 0.62 | 0.63 |
| PSSI | 1.2 | 1.3 |

From Table 7 it can be seen that the polymers prepared according to the present invention lead to very good values in KV₄₀, HTHS₈₀ and HTHS₁₀₀. Low viscosity values in KV₄₀, HTHS₈₀ and HTHS₁₀₀ are used as an indication for good fuel efficiency (see US 2010/0190671). It can therefore be expected that these polymers lead to improved fuel economy by additionally providing a dispersant functionality at very good HAZE levels even when produced in a sequential manner.

As a conclusion, the data presented above show that the method according to the present invention for producing polyalkyl (meth)acrylates, wherein the amounts of the different monomers are split into a heel and one or more feeds with different compositions and concentrations, results in the formation of a higher amount of polymers having a composition closer to the average polymer composition throughout the whole polymerization process.

This approach leads to products with reduced HAZE (marker for the solubility of the polymer in a given base oil) and therefore improved solubility of the polymers in lubricant formulations, especially in engine oil formulations, improved up-scalability and very good viscometric properties at the same time.

## Claims

1. Method for the preparation of polyalkyl (meth)acrylate polymers consisting of:
(a) 10 to 20% by weight of esters of (meth)acrylic acid and a hydroxylated hydrogenated polybutadiene;
(b1) 45% to 60% by weight of C₁₋₄ alkyl (meth)acrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N-containing monomers selected from the group consisting of N,N-dimethylaminoethyl methacrylate (DMAEMA), N-(3-(dimethylamino)propyl)methacrylamide (DMAPMAm) and N-vinylpyrrolidinone (NVP), preferably DMAEMA,
based on the total amount of the polyalkyl (meth)acrylate polymers,
the method comprising the steps of:
(i) preparing a monomer mixture 1 comprising 130 to 145% of the targeted content of monomers (a) and 90% to 96% of the targeted content of monomers (b), the concentration of the monomers in mixture **1** being 50 to 60%;
(ii) adding a monomer mixture **2** comprising 50 to 60% of the targeted content of monomers (a) and 105% to 110% of the targeted content of monomers (b), the concentration of the monomers in mixture **2** being 50 to 60%;
**characterized in that** monomer mixture **1** comprises 50 to 60% of the total amount of monomers used in the process and monomer mixture **2** comprises 40 to 50% of the total amount of monomers used in the process.

2. The method according to claim 1, wherein the monomer mixture **2** can be further split into monomer mixture **2a** and monomer mixture **2b,** wherein
mixture **2a** comprises 100% of the targeted content of monomers (a) and 100% of the targeted content of monomers (b), the concentration of the monomers in mixture **2a** being 50 to 60% and
monomer mixture 2b comprises 0% of the targeted content of monomers (a) and 115-125% of the targeted content of monomers (b), the concentration of the monomers in mixture **2b** being 50 to 60%,
**characterized in that** monomer mixture **2a** comprises 20 to 30% of the total amount of monomers used in the process, and monomer mixture **2b** comprises 20 to 25% of the total amount of monomers used in the process.

3. The method according to any one of the preceding claims, wherein the polyalkyl (meth)acrylate polymer consists of:
(a) 10 to 20% by weight of esters of (meth)acrylic acid and a hydroxylated hydrogenated polybutadiene;
(b1) 45% to 60% by weight of C₁₋₄ alkyl methacrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N,N-dimethylaminoethyl methacrylate (DMAEMA).

4. The method according to any one of the preceding claims, wherein the weight-average molecular weight of the polyalkyl(meth)acrylate polymers is in the range of 100,000 to 1,000,000 g/mol, preferably in the range of 400,000 to 700,000 g/mol.

5. The method according to any one of the preceding claims, wherein the monomer mixtures further comprise a base oil selected from the group consisting of API Group I, II, III, IV or V oils and mixtures thereof.

6. The method according to any one of the preceding claims, wherein the monomer mixtures further comprise a base oil that comprises a mixture of API Group III and API Group V oils.

7. The method according to any one of the preceding claims, wherein
mixture **1** comprises 60% to 75% by weight of API Group III oil or mixtures thereof and 25% to 40% by weight of Group V base oil and mixtures thereof, and
mixture **2** comprises 75% to 85% by weight of API Group III oil or mixtures thereof and 15% to 25% by weight of Group V base oil and mixtures thereof; or
mixture **1** comprises 65% to 75% by weight of API Group III oil or mixtures thereof and 25% to 35% by weight of Group V base oil and mixtures thereof, and
mixture **2a** comprises 65% to 75% by weight of API Group III oil or mixtures thereof and 25% to 35% by weight of Group V base oil and mixtures thereof, and
mixture **2b** comprises 65% to 75% by weight of API Group III oil or mixtures thereof and 25% to 35% by weight of Group V base oil and mixtures thereof,
based on the total weight of the base oil.

8. Method for the preparation of polyalkyl (meth)acrylate polymers, wherein the polyalkyl (meth)acrylate polymer consists of:
(a) 10 to 20% by weight of esters of (meth)acrylic acid and a hydroxylated hydrogenated polybutadiene;
(b1) 45% to 60% by weight of C₁₋₄ alkyl (meth)acrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N-containing monomers selected from the group consisting of N,N-dimethylaminoethyl methacrylate (DMAEMA), N-(3-(dimethylamino)propyl)methacrylamide (DMAPMAm) and N-vinylpyrrolidinone (NVP), preferably DMAEMA,
based on the total amount of the polyalkyl (meth)acrylate polymers,
the method comprising the steps of:
(i) preparing a monomer mixture **1** comprising 18 to 23% by weight of monomers (a), 45% to 52% by weight of monomers (b1), 14% to 18% by weight of monomers (b2), 9% to 11% by weight of monomers (b3) and 2.5 to 6.5% by weight of monomers (b4), based on the total amount of monomers in mixture 1, in a base oil, the concentration of the monomers in mixture **1** being 50 to 60%; and
(ii) adding a monomer mixture **2** comprising 6 to 11% by weight of monomers (a), 53% to 60% by weight of monomers (b1), 16 to 20% by weight of monomers (b2), 10 to 13% by weight of monomers (b3) and 3 to 7% by weight of monomers (b4), based on the total amount of monomers in mixture **2**, in a base oil, the concentration of the monomers in mixture **2** being 50 to 60%;
**characterized in that** monomer mixture **1** comprises 54 to 59% of the total amount of monomers used in the process and monomer mixture **2** comprises 41 to 46% of the total amount of monomers used in the process, or
(ii) adding a monomer mixture **2a** comprising 13 to 17% by weight of monomers (a), 49% to 55% by weight of monomers (b1), 15 to 19% by weight of monomers (b2), 10 to 12% by weight of monomers (b3) and 2.5 to 7% by weight of monomers (b4), based on the total amount of monomers in mixture **2a,** in a base oil, the concentration of the monomers in mixture **2a** being 53 to 57%; and
(iii) adding a monomer mixture **2b** comprising 0 to 1% by weight of monomers (a), 58% to 65% by weight of monomers (b1), 18 to 22% by weight of monomers (b2), 12 to 14% by weight of monomers (b3) and 3 to 8% by weight of monomers (b4), based on the total amount of monomers in mixture **2b,** in a base oil, the concentration of the monomers in mixture **2b** being 51 to 55%.
**characterized in that** monomer mixture **2a** comprises 23 to 27% of the total amount of monomers used in the process and monomer mixture **2b** comprises 20 to 24% of the total amount of monomers used in the process wherein
mixture **1** comprises 60% to 75% by weight of API Group III oil or mixtures thereof and 25% to 40% by weight of Group V base oil and mixtures thereof, based on the total amount of base oil used in mixture **1;** and
mixture **2** comprises 75% to 85% by weight of API Group III oil or mixtures thereof and 15% to 25% by weight of Group V base oil and mixtures thereof, based on the total amount of base oil used in mixture **2;** or
mixture **1** comprises 65% to 75% by weight of API Group III oil or mixtures thereof and 25% to 35% by weight of Group V base oil and mixtures thereof, based on the total amount of base oil used in mixture **1;**
mixture **2a** comprises 65% to 75% by weight of API Group III oil or mixtures thereof and 25% to 35% by weight of Group V base oil and mixtures thereof, based on the total amount of base oil used in mixture **2a;** and
mixture **2b** comprises 65% to 75% by weight of API Group III oil or mixtures thereof and 25% to 35% by weight of Group V base oil and mixtures thereof, based on the total amount of base oil used in mixture **2b**.

9. The method according to claim 8, wherein the polyalkyl (meth)acrylate polymer consists of:
(a) 10 to 20% by weight of esters of methacrylic acid and a hydroxylated hydrogenated polybutadiene;
(b1) 45% to 60% by weight of C₁₋₄ alkyl methacrylates;
(b2) 10% to 25% by weight of C₁₀₋₁₅ alkyl methacrylates, more preferably C₁₂₋₁₄ alkyl methacrylates;
(b3) 10% to 15% by weight of styrene; and
(b4) 5% to 7% by weight of N,N-dimethylaminoethyl methacrylate (DMAEMA).

## Patentansprüche

1. Verfahren zur Herstellung von Polyalkyl(meth)acrylat-Polymeren, bestehend aus:
(a) 10 bis 20 Gew.-% Estern von (Meth)acrylsäure und einem hydroxylierten hydrierten Polybutadien;
(b1) 45 bis 60 Gew.-% C₁₋₄-Alkyl (meth) acrylaten;
(b2) 10 bis 25 Gew.-% C₁₀₋₁₅-Alkylmethacrylaten, weiter bevorzugt C₁₂₋₁₄-Alkylmethacrylaten;
(b3) 10 bis 15 Gew.-% Styrol und
(b4) 5 bis 7 Gew.-% von N-haltigen Monomeren, ausgewählt aus der Gruppe bestehend aus N,N-Dimethylaminoethylmethacrylat (DMAEMA), N-(3-(Dimethylamino)propyl)methacrylamid (DMAPMAm) und N-Vinylpyrrolidinon (NVP), vorzugsweise DMAEMA,
bezogen auf die Gesamtmenge der Polyalkyl(meth)acrylat-Polymere,
wobei das Verfahren folgende Schritte umfasst:
(i) Herstellen einer Monomerenmischung 1, umfassend 130 bis 145 % des angestrebten Gehalts von Monomeren (a) und 90 % bis 96 % des angestrebten Gehalts von Monomeren (b), wobei die Konzentration der Monomere in der Mischung 1 50 bis 60 % beträgt;
(ii) Zugeben einer Monomerenmischung 2, umfassend 50 bis 60 % des angestrebten Gehalts von Monomeren (a) und 105 % bis 110 % des angestrebten Gehalts von Monomeren (b), wobei die Konzentration der Monomere in der Mischung 2 50 bis 60 % beträgt;
**dadurch gekennzeichnet, dass** die Monomerenmischung 1 50 bis 60 % der Gesamtmenge der bei dem Verfahren verwendeten Monomere umfasst und die Monomerenmischung 2 40 bis 50 % der Gesamtmenge der bei dem Verfahren verwendeten Monomere umfasst.

2. Verfahren nach Anspruch 1, wobei die Monomerenmischung 2 ferner in Monomerenmischung 2a und Monomerenmischung 2b aufgeteilt werden kann, wobei
Mischung 2a 100 % des angestrebten Gehalts von Monomeren (a) und 100 % des angestrebten Gehalts von Monomeren (b) umfasst, wobei die Konzentration der Monomere in der Mischung 2a 50 bis 60 % beträgt, und
Monomerenmischung 2b 0 % des angestrebten Gehalts von Monomeren (a) und 115-125 % des angestrebten Gehalts von Monomeren (b) umfasst, wobei die Konzentration der Monomere in der Mischung 2b 50 bis 60 % beträgt,
**dadurch gekennzeichnet, dass** die Monomerenmischung 2a 20 bis 30 % der Gesamtmenge der bei dem Verfahren verwendeten Monomere umfasst und die Monomerenmischung 2b 20 bis 25 % der Gesamtmenge der bei dem Verfahren verwendeten Monomere umfasst.

3. Verfahren nach einem der vorhergehenden Ansprüche, wobei das Polyalkyl(meth)acrylat-Polymer aus Folgendem besteht:
(a) 10 bis 20 Gew.-% Estern von (Meth)acrylsäure und einem hydroxylierten hydrierten Polybutadien;
(b1) 45 bis 60 Gew.-% C₁₋₄-Alkylmethacrylaten;
(b2) 10 bis 25 Gew.-% C₁₀₋₁₅-Alkylmethacrylaten, weiter bevorzugt C₁₂₋₁₄-Alkylmethacrylaten;
(b3) 10 bis 15 Gew.-% Styrol und
(b4) 5 bis 7 Gew.-% N,N-Dimethylaminoethylmethacrylat (DMAEMA).

4. Verfahren nach einem der vorhergehenden Ansprüche, wobei das gewichtsmittlere Molekulargewicht der Polyalkyl(meth)acrylat-Polymere im Bereich von 100.000 bis 1.000.000 g/mol, vorzugsweise im Bereich von 400.000 bis 700.000 g/mol, liegt.

5. Verfahren nach einem der vorhergehenden Ansprüche, wobei die Monomerenmischungen ferner ein Grundöl aus der Gruppe bestehend aus Ölen der API-Gruppe I, II, III, IV oder V und Mischungen davon umfassen.

6. Verfahren nach einem der vorhergehenden Ansprüche, wobei die Monomerenmischungen ferner ein Grundöl umfassen, welches eine Mischung von Ölen der API-Gruppe III und API-Gruppe V umfasst.

7. Verfahren nach einem der vorhergehenden Ansprüche, wobei
Mischung 1 60 bis 75 Gew.-% Öl der API-Gruppe III oder Mischungen davon und 25 bis 40 Gew.-% Grundöl der Gruppe V und Mischungen davon umfasst und
Mischung 2_ 75 bis 85 Gew.-% Öl der API-Gruppe III oder Mischungen davon und 15 bis 25 Gew.-% Grundöl der Gruppe V und Mischungen davon umfasst oder
Mischung 1 65 bis 75 Gew.-% Öl der API-Gruppe III oder Mischungen davon und 25 bis 35 Gew.-% Grundöl der Gruppe V und Mischungen davon umfasst und
Mischung 2a 65 bis 75 Gew.-% Öl der API-Gruppe III oder Mischungen davon und 25 bis 35 Gew.-% Grundöl der Gruppe V und Mischungen davon umfasst und
Mischung 2b 65 bis 75 Gew.-% Öl der API-Gruppe III oder Mischungen davon und 25 bis 35 Gew.-% Grundöl der Gruppe V und Mischungen davon umfasst,
bezogen auf das Gesamtgewicht des Grundöls.

8. Verfahren zur Herstellung von Polyalkyl(meth)acrylat-Polymeren, wobei das Polyalkyl(meth)acrylat-Polymer aus Folgendem besteht:
(a) 10 bis 20 Gew.-% Estern von (Meth)acrylsäure und einem hydroxylierten hydrierten Polybutadien;
(b1) 45 bis 60 Gew.-% C₁₋₄-Alkyl (meth) acrylaten;
(b2) 10 bis 25 Gew.-% C₁₀₋₁₅-Alkylmethacrylaten, weiter bevorzugt C₁₂₋₁₄-Alkylmethacrylaten;
(b3) 10 bis 15 Gew.-% Styrol und
(b4) 5 bis 7 Gew.-% von N-haltigen Monomeren, ausgewählt aus der Gruppe bestehend aus N,N-Dimethylaminoethylmethacrylat (DMAEMA), N-(3-(Dimethylamino)propyl)methacrylamid (DMAPMAm) und N-Vinylpyrrolidinon (NVP), vorzugsweise DMAEMA,
bezogen auf die Gesamtmenge der Polyalkyl(meth)acrylat-Polymere,
wobei das Verfahren folgende Schritte umfasst:
(i) Herstellen einer Monomerenmischung 1, umfassend 18 bis 23 Gew.-% Monomere (a), 45 bis 52 Gew.-% Monomere (b1), 14 bis 18 Gew.-% Monomere (b2), 9 bis 11 Gew.-% Monomere (b3) und 2,5 bis 6,5 Gew.-% Monomere (b4), bezogen auf die Gesamtmenge von Monomeren in der Mischung 1, in einem Grundöl, wobei die Konzentration der Monomere in der Mischung 1 50 bis 60 % beträgt; und
(ii) Zugeben einer Monomerenmischung 2, umfassend 6 bis 11 Gew.-% Monomere (a), 53 bis 60 Gew.-% Monomere (b1), 16 bis 20 Gew.-% Monomere (b2), 10 bis 13 Gew.-% Monomere (b3) und 3 bis 7 Gew.-% Monomere (b4), bezogen auf die Gesamtmenge von Monomeren in der Mischung 2, in einem Grundöl, wobei die Konzentration der Monomere in der Mischung 2 50 bis 60 % beträgt;
**dadurch gekennzeichnet, dass** die Monomerenmischung 1. 54 bis 59 % der Gesamtmenge der bei dem Verfahren verwendeten Monomere umfasst und die Monomerenmischung 2 41 bis 46 % der Gesamtmenge der bei dem Verfahren verwendeten Monomere umfasst, oder
(ii) Zugeben einer Monomerenmischung 2a, umfassend 13 bis 17 Gew.-% Monomere (a), 49 bis 55 Gew.-% Monomere (b1), 15 bis 19 Gew.-% Monomere (b2), 10 bis 12 Gew.-% Monomere (b3) und 2,5 bis 7 Gew.-% Monomere (b4), bezogen auf die Gesamtmenge von Monomeren in der Mischung 2a, in einem Grundöl, wobei die Konzentration der Monomere in der Mischung 2a 53 bis 57 % beträgt; und
(iii)Zugeben einer Monomerenmischung 2b, umfassend 0 bis 1 Gew.-% Monomere (a), 58 bis 65 Gew.-% Monomere (b1), 18 bis 22 Gew.-% Monomere (b2), 12 bis 14 Gew.-% Monomere (b3) und 3 bis 8 Gew.-% Monomere (b4), bezogen auf die Gesamtmenge von Monomeren in der Mischung 2b, in einem Grundöl, wobei die Konzentration der Monomere in der Mischung 2b 51 bis 55 % beträgt,
**dadurch gekennzeichnet dass** die Monomerenmischung 2a 23 bis 27 % der Gesamtmenge der bei dem Verfahren verwendeten Monomere umfasst und die Monomerenmischung 2b 20 bis 24 % der Gesamtmenge der bei dem Verfahren verwendeten Monomere umfasst, wobei
Mischung 1 60 bis 75 Gew.-% Öl der API-Gruppe III oder Mischungen davon und 25 bis 40 Gew.-% Grundöl der Gruppe V und Mischungen davon, bezogen auf die Gesamtmenge des in Mischung 1 verwendeten Grundöls, umfasst und
Mischung 2 75 bis 85 Gew.-% Öl der API-Gruppe III oder Mischungen davon und 15 bis 25 Gew.-% Grundöl der Gruppe V und Mischungen davon, bezogen auf die Gesamtmenge des in Mischung 2 verwendeten Grundöls, umfasst oder
Mischung 1 65 bis 75 Gew.-% Öl der API-Gruppe III oder Mischungen davon und 25 bis 35 Gew.-% Grundöl der Gruppe V und Mischungen davon, bezogen auf die Gesamtmenge des in Mischung 1 verwendeten Grundöls, umfasst;
Mischung 2a 65 bis 75 Gew.-% Öl der API-Gruppe III oder Mischungen davon und 25 bis 35 Gew.-% Grundöl der Gruppe V und Mischungen davon, bezogen auf die Gesamtmenge des in Mischung 2a verwendeten Grundöls, umfasst und
Mischung 2b 65 bis 75 Gew.-% Öl der API-Gruppe III oder Mischungen davon und 25 bis 35 Gew.-% Grundöl der Gruppe V und Mischungen davon, bezogen auf die Gesamtmenge des in Mischung 2b verwendeten Grundöls, umfasst.

9. Verfahren nach Anspruch 8, wobei das Polyalkyl(meth)acrylat-Polymer aus Folgendem besteht:
(a) 10 bis 20 Gew.-% Estern von Methacrylsäure und einem hydroxylierten hydrierten Polybutadien;
(b1) 45 bis 60 Gew.-% C₁₋₄-Alkylmethacrylaten;
(b2) 10 bis 25 Gew.-% C₁₀₋₁₅-Alkylmethacrylaten, weiter bevorzugt C₁₂₋₁₄-Alkylmethacrylaten;
(b3) 10 bis 15 Gew.-% Styrol und
(b4) 5 bis 7 Gew.-% N,N-Dimethylaminoethylmethacrylat (DMAEMA).

## Revendications

1. Procédé pour la préparation de polymères de type poly((méth)acrylate d'alkyle) constitués de :
(a) 10 à 20% en poids d'esters d'acide (méth)acrylique et d'un polybutadiène hydrogéné hydroxylé;
(b1) 45% à 60% en poids de (méth)acrylates de C₁₋₄ alkyle;
(b2) 10% à 25% en poids de méthacrylates de C₁₀₋₁₅ alkyle, plus préférablement de méthacrylates de C₁₂₋₁₄ alkyle;
(b3) 10% à 15% en poids de styrène; et
(b4) 5% à 7% en poids de monomères contenant N choisis dans le groupe constitué par méthacrylate de N,N-diméthylaminoéthyle (DMAEMA), N-(3-(diméthylamino)propyl)méthacrylamide (DMAPMAm) et N-vinylpyrrolidinone (NVP), de préférence DMAEMA,
sur la base de la quantité totale des polymères de type poly((méth)acrylate d'alkyle),
le procédé comprenant les étapes de:
(i) préparation d'un mélange de monomères 1 comprenant 130 à 145% de la teneur cible de monomères (a) et 90% à 96% de la teneur cible de monomères (b), la concentration des monomères dans le mélange 1 étant de 50 à 60%;
(ii) ajout d'un mélange de monomères 2 comprenant 50 à 60% de la teneur cible de monomères (a) et 105% à 110% de la teneur cible de monomères (b), la concentration des monomères dans le mélange 2_ étant de 50 à 60%;
**caractérisé en ce que** le mélange de monomères 1 comprend 50 à 60% de la quantité totale de monomères utilisés dans le processus et le mélange de monomères 2 comprend 40 à 50% de la quantité totale de monomères utilisés dans le processus.

2. Procédé selon la revendication 1, dans lequel le mélange de monomères 2_ peut être en outre divisé en un mélange de monomères 2a et un mélange de monomères 2b, dans lequel
le mélange 2a comprend 100% de la teneur cible de monomères (a) et 100% de la teneur cible de monomères (b), la concentration des monomères dans le mélange 2a étant de 50 à 60%, et
le mélange de monomères 2b comprend 0% de la teneur cible de monomères (a) et 115 à 125% de la teneur cible de monomères (b), la concentration des monomères dans le mélange 2b étant de 50 à 60%, **caractérisé en ce que** le mélange de monomères 2a comprend 20 à 30% de la quantité totale de monomères utilisés dans le processus, et le mélange de monomères 2b comprend 20 à 25% de la quantité totale de monomères utilisés dans le processus.

3. Procédé selon l'une quelconque des revendications précédentes, dans lequel le polymère de type poly((méth)acrylate d'alkyle) est constitué de:
(a) 10 à 20% en poids d'esters d'acide (méth)acrylique et d'un polybutadiène hydrogéné hydroxylé;
(b1) 45% à 60% en poids de méthacrylates de C₁₋₄ alkyle;
(b2) 10% à 25% en poids de méthacrylates de C₁₀₋₁₅ alkyle, plus préférablement de méthacrylates de C₁₂₋₁₄ alkyle;
(b3) 10% à 15% en poids de styrène; et
(b4) 5% à 7% en poids de méthacrylate de N,N-diméthylaminoéthyle (DMAEMA).

4. Procédé selon l'une quelconque des revendications précédentes, le poids moléculaire moyen en poids des polymères de type poly((méth)acrylate d'alkyle) étant dans la plage de 100 000 à 1 000 000 g/mole, préférablement dans la plage de 400 000 à 700 000 g/mole.

5. Procédé selon l'une quelconque des revendications précédentes, les mélanges de monomères comprenant en outre une huile de base choisie dans le groupe constitué par des huiles du groupe I, II, III, IV ou V de l'API et des mélanges correspondants.

6. Procédé selon l'une quelconque des revendications précédentes, les mélanges de monomères comprenant en outre une huile de base qui comprend un mélange d'huiles du groupe III de l'API et du groupe V de l'API.

7. Procédé selon l'une quelconque des revendications précédentes,
le mélange 1 comprenant 60% à 75% en poids d'huile du groupe III de l'API ou des mélanges correspondants et 25% à 40% en poids d'huile de base du groupe V et des mélanges correspondants, et
le mélange 2 comprenant 75% à 85% en poids d'huile du groupe III de l'API ou des mélanges correspondants et 15% à 25% en poids d'huile de base du groupe V et des mélanges correspondants; ou
le mélange 1 comprenant 65% à 75% en poids d'huile du groupe III de l'API ou des mélanges correspondants et 25% à 35% en poids d'huile de base du groupe V et des mélanges correspondants, et
le mélange 2a comprenant 65% à 75% en poids d'huile du groupe III de l'API ou des mélanges correspondants et 25% à 35% en poids d'huile de base du groupe V et des mélanges correspondants, et
le mélange 2b comprenant 65% à 75% en poids d'huile du groupe III de l'API ou des mélanges correspondants et 25% à 35% en poids d'huile de base du groupe V et des mélanges correspondants,
sur la base du poids total de l'huile de base.

8. Procédé pour la préparation de polymères de type poly((méth)acrylate d'alkyle), le polymère de type poly((méth)acrylate d'alkyle) étant constitué de :
(a) 10 à 20% en poids d'esters d'acide (méth)acrylique et d'un polybutadiène hydrogéné hydroxylé;
(b1) 45% à 60% en poids de (méth)acrylates de C₁₋₄ alkyle;
(b2) 10% à 25% en poids de méthacrylates de C₁₀₋₁₅ alkyle, plus préférablement de méthacrylates de C₁₂₋₁₄ alkyle;
(b3) 10% à 15% en poids de styrène; et
(b4) 5% à 7% en poids de monomères contenant N choisis dans le groupe constitué par méthacrylate de N,N-diméthylaminoéthyle (DMAEMA), N-(3-(diméthylamino)propyl)méthacrylamide (DMAPMAm) et N-vinylpyrrolidinone (NVP), de préférence DMAEMA,
sur la base de la quantité totale des polymères de type poly((méth)acrylate d'alkyle),
le procédé comprenant les étapes de:
(i) préparation d'un mélange de monomères 1 comprenant 18 à 23% en poids de monomères (a), 45% à 52% en poids de monomères (b1), 14% à 18% en poids de monomères (b2), 9% à 11% en poids de monomères (b3) et 2,5 à 6,5% en poids de monomères (b4), sur la base de la quantité totale de monomères dans le mélange 1, dans une huile de base, la concentration des monomères dans le mélange 1 étant de 50 à 60%; et
(ii) ajout d'un mélange de monomères 2 comprenant 6% à 11% en poids de monomères (a), 53% à 60% en poids de monomères (b1), 16 à 20% en poids de monomères (b2), 10 à 13% en poids de monomères (b3) et 3 à 7% en poids de monomères (b4), sur la base de la quantité totale de monomères dans le mélange 2, dans une huile de base, la concentration des monomères dans le mélange 2 étant de 50 à 60%;
**caractérisé en ce que** le mélange de monomères 1 comprend 54 à 59% de la quantité totale de monomères utilisés dans le processus et le mélange de monomères 2 comprend 41 à 46% de la quantité totale de monomères utilisés dans le processus, ou
(ii) ajout d'un mélange de monomères 2a comprenant 13 à 17% en poids de monomères (a), 49% à 55% en poids de monomères (b1), 15 à 19% en poids de monomères (b2), 10 à 12% en poids de monomères (b3) et 2,5% à 7% en poids de monomères (b4), sur la base de la quantité totale de monomères dans le mélange 2a, dans une huile de base, la concentration des monomères dans le mélange 2a étant de 53 à 57%; et
(iii) ajout d'un mélange de monomères 2b comprenant 0% à 1% en poids de monomères (a), 58% à 65% en poids de monomères (b1), 18% à 22% en poids de monomères (b2), 12 à 14% en poids de monomères (b3) et 3% à 8% en poids de monomères (b4), sur la base de la quantité totale de monomères dans le mélange 2b, dans une huile de base, la concentration des monomères dans le mélange 2b étant de 51 à 55%; et
**caractérisé en ce que** le mélange de monomères 2a comprend 23 à 27% de la quantité totale de monomères utilisés dans le processus et le mélange de monomères 2b comprend 20 à 24% de la quantité totale de monomères utilisés dans le processus dans lequel
le mélange 1 comprend 60% à 75% en poids d'huile du groupe III de l'API ou des mélanges correspondants et 25% à 40% en poids d'huile de base du groupe V et des mélanges correspondants, sur la base de la quantité totale d'huile de base utilisée dans le mélange 1; et
le mélange 2 comprend 75% à 85% en poids d'huile du groupe III de l'API ou des mélanges correspondants et 15% à 25% en poids d'huile de base du groupe V et des mélanges correspondants, sur la base de la quantité totale d'huile de base utilisée dans le mélange 2; ou
le mélange 1 comprend 65% à 75% en poids d'huile du groupe III de l'API ou des mélanges correspondants et 25% à 35% en poids d'huile de base du groupe V et des mélanges correspondants, sur la base de la quantité totale d'huile de base utilisée dans le mélange 1;
le mélange 2a comprend 65% à 75% en poids d'huile du groupe III de l'API ou des mélanges correspondants et 25% à 35% en poids d'huile de base du groupe V et des mélanges correspondants, sur la base de la quantité totale d'huile de base utilisée dans le mélange 2a; et
le mélange 2b comprend 65% à 75% en poids d'huile du groupe III de l'API ou des mélanges correspondants et 25% à 35% en poids d'huile de base du groupe V et des mélanges correspondants, sur la base de la quantité totale d'huile de base utilisée dans le mélange 2b.

9. Procédé selon la revendication 8, le polymère de type poly((méth)acrylate d'alkyle) étant constitué de:
(a) 10 à 20% en poids d'esters d'acide méthacrylique et d'un polybutadiène hydrogéné hydroxylé;
(b1) 45% à 60% en poids de méthacrylates de C₁₋₄ alkyle;
(b2) 10% à 25% en poids de méthacrylates de C₁₀₋₁₅ alkyle, plus préférablement de méthacrylates de C₁₂₋₁₄ alkyle;
(b3) 10% à 15% en poids de styrène; et
(b4) 5% à 7% en poids de méthacrylate de N,N-diméthylaminoéthyle (DMAEMA).
